# EUROPEAN PATENT SPECIFICATION

(11) **EP 2 220 295 B1**
(45) Date of publication and mention of the grant of the patent: **22.05.2019**
(21) Application number: 08847575.1
(22) Date of filing: 07.11.2008
(51) Int. Cl.: E06B 3/70, E06B 3/48, E06B 3/58, B27N 1/00, B27N 3/08, B27N 3/20

(54) **THIN-LAYER LIGNOCELLULOSIC COMPOSITE HAVING INCREASED RESISTANCE TO MOISTURE AND METHODS OF MAKING THE SAME**
DÜNNSCHICHTIGER LIGNOZELLULOSEVERBUNDSTOFF MIT ERHÖHTER FEUCHTIGKEITSRESISTENZ UND HERSTELLUNGSVERFAHREN DAFÜR
COMPOSITE LIGNOCELLULOSIQUE EN COUCHE MINCE AYANT UNE RÉSISTANCE ACCRUE À L'HUMIDITÉ ET SON PROCÉDÉ DE FABRICATION

(30) Priority: 07.11.2007 US 983090; 07.11.2007 US 983091
(43) Date of publication of application: 25.08.2010
(73) Proprietor: Jeld-Wen, Inc., Klamath Falls, OR 97601 (US)
(72) Inventor: CLARK, Randy J., Klamath Falls, Oregon 97601 (US); KIEST, Kenneth D., Klamath Falls, Oregon 97603 (US)
(74) Representative: Phillips & Leigh LLP
(86) International application number: PCT/US2008/012576
(87) International publication number: WO 2009/061474

(56) References cited:
- EP-B- 0 909 295
- EP-B- 0 909 295
- EP-B- 0 909 295
- WO-A-2004/076141
- WO-A1-98/32600
- WO-A1-98/32600
- WO-A2-2004/076141
- WO-A2-2004/076141
- US-A- 5 344 484
- US-A- 5 344 484
- US-A- 5 344 484
- US-A1- 2006 272 253
- US-A1- 2006 272 253

## Description

### BACKGROUND OF THE INVENTION

The present invention relates to the manufacture of thin-layer lignocellulosic composites, such as interior and/or exterior wood-based doorskins. More particularly, the present invention relates to thin-layer wood composites that include an isocyanate based-resin and thus, exhibit significantly less swelling and/or shrinking upon exposure to the environment.

Doors manufactured from wood have a pleasing appearance and a substantial and solid feel. While the appearance of natural wood is aesthetically pleasing, wood can be susceptible to damage caused by long-term exposure to humid or dry air, weather, fungal infestation, and insect pests. Thus, frequent and often costly maintenance may be required to prevent the deterioration of finished wood that is exposed to the environment. Also, many species of wood having a desirable appearance are also expensive, and require significant labor and time for production of finished articles.

Metal doors may be more cost-effective than wood to manufacture and maintain, but may not be as aesthetically pleasing to the consumer. For example, metal garage doors may only be available in limited color lines and often do not simulate a natural wood grain in a very realistic manner. Also, metal garage doors may be limited in design, in that it may be difficult to add three dimensional shaping, such as trim or paneling, to the outer surface of a metal door. For example, some manufacturers apply extrusive plastic panels to the face of a metal garage door to add a design to the face of the door. The plastic and metal components, however, may exhibit different physical properties in response to changes in temperature and humidity and thus, the door may exhibit warping or other types of deformation upon exposure to weather.

A significant problem in the manufacture of wood-based composite products that are exposed to the exterior and extreme interior environments is that upon exposure to variations in temperature and moisture, the wood can lose water and shrink, or gain water and swell. This tendency to shrink and/or swell can significantly limit the useful lifetime of most exterior wood products, such as wooden doors, often necessitating replacement after only a few years. The problem is particularly prevalent in areas of high moisture (e.g., Hawaii) or in climates that are extremely hot or dry (e.g., Arizona). Shrinking and swelling can also be a problem when the wood is exposed to a wet environment during construction, or upon exposure to the dry heat used indoors in the winter.

A possible solution to the problem of moisture gain and loss in wood exposed to the elements includes covering the wood with paint and/or other coatings that act as a barrier to moisture. Still, such coatings tend to wear off with time, leaving the wood susceptible to the environment.

Rather than treating the unit at the site of installation, it may be preferable to manufacture products that exhibit increased resistance to moisture gain and loss. For example, increasing the amounts of resin content or decreasing the amount of wood fiber used in a door can increase resistance to water gain and water loss. Such modifications, however, can be associated with significantly increased production challenges. Other options include the use of metal or fiberglass doors, but such doors are not always as aesthetically pleasing as wood doors and may have other performance problems associated with the use of these materials.

Alternatively, doors, and other structural units, may be constructed with a wood-composite water-resistant layer. For example, doors may be covered with a thin-layer wood composite known as a doorskin. Generally, doorskins are molded as thin layers and secured to an underlying door frame to thereby provide a water-resistant outer surface. Doorskins may be made by mixing wood fiber, wax, and a resin binder, and then pressing the mixture under conditions of elevated temperature and pressure to form a thin-layer wood composite that may then be bonded to the underlying door frame. Wood composite doorskins are traditionally formed by pressing wood fragments in the presence of a binder at temperatures exceeding 275 °F (135 °C). The resin binder used in the doorskin may be a formaldehyde-based resin, an isocyanate-based resin, or other thermoplastic or thermoset resins. Formaldehyde-based resins typically used to make wood composite products include phenol-formaldehyde, urea-formaldehyde, or melamine-formaldehyde resins. Phenol-formaldehyde resins require a high temperature cure and are sensitive to the amount of water in the wood since excess water can inhibit the high temperature cure. Urea and melamine-formaldehyde resins do not require as high of a temperature cure, but traditionally do not provide comparable water-resistance (at the same resin content) in the doorskin product.

Additionally, many states are regulating the use of formaldehyde- based products due to environmental and health concerns related to reported carcinogenic effects of formaldehyde. Accordingly, formaldehyde-based products are losing favor in the market, and in some cases are regulated, and in other cases, banned from the market.

As compared to doorskins made using phenol-formaldehyde resins, doorskins that utilize high-temperature pressed isocyanate resin binder display increased surface strength. These doorskins, however, exhibit decreased porosity to adhesives and thus, do not bond well to the underlying doorframe. Also, isocyanate-bonded wood composites made using currently available methods and compositions do not consistently exhibit sufficient resistance to environmentally-induced swelling and/or shrinking to be commercially useful. WO2004/076141 concerns thin-layer lignocellulose composites having increased resistance to moisture. The composites are formed from a mixture including a refined lignocellulosic fiber, wax and an organic isocyanate resin, initially pressed to form a loose mat. A release agent is included as a part of the fiber mixture, or sprayed onto the surface of the mat. A surface of the die used to press the mat may be coated with an anti-bonding agent.

### SUMMARY OF THE INVENTION

The present invention provides a method of producing a thin-layer lignocellulosic composite having increased resistance to moisture-induced shrinking or swelling, as defined in claim 1. The invention correspondingly provides a thin-layer lignocellulosic composite as defined in claim 5.

The mixture may comprise a release agent, and a tackifier, wherein the mixture is substantially free of added wax. The mixture is pressed between two dies at an elevated temperature and pressure and for a sufficient time to form a thin-layer composite of predetermined thickness, and to allow the isocyanate resin to interact with the lignocellulosic fiber such that the resultant thin-layer composite has a predetermined resistance to moisture.

It is to be understood that the invention is not limited in its application to the specific details as set forth in the following description, figures and claims. The invention is capable of other embodiments and of being practiced or carried out in various ways.

### BRIEF DESCRIPTION OF THE FIGURES

Figure 1 illustrates an embodiment of a method that may be used to make a thin-layer wood composite doorskin.
Figure 2 illustrates an embodiment of a method used to make water-resistant thin-layer wood composites in accordance with an embodiment of the present invention where panel (a) shows mixing of the lignocellulosic fiber and resin; panel (b) shows forming the composite into a loose formed mat; panel (c) shows spraying the loose formed mat with release agent; panel (d) shows pressing the mat between two dies; and panel (e) shows the resultant thin-layered composite product.
Figure 3 illustrates a perspective view of a composite single car garage door in accordance with an illustrative embodiment of the present invention with enlargements of indicated portions of the door shown in Fig. 3A and Fig. 3B.
Figure 4 illustrates a front view of a composite single car garage door in accordance with an illustrative embodiment of the present invention.
Figure 5 illustrates a perspective view of a composite two car garage door in accordance with an illustrative embodiment of the present invention.
Figure 6 illustrates a composite two car garage door in accordance with an enlargement of the indicated region shown in Fig. 6A.
Figure 7 illustrates a composite two car garage door in accordance with an illustrative embodiment of the present invention with an enlargement of the indicated region shown in Fig. 7A.
Figure 8 illustrates a perspective view of various components used to make a composite garage door in accordance with an illustrative embodiment of the present invention.
Figures 9A and 9B illustrate an embodiment of a process used to manufacture single car composite garage door panels in accordance with the present invention, where Fig. 9A illustrates a process used to make a flush door panel, and Fig. 9B illustrates processes used to add raised surfaces to flush door panels.

### DETAILED DESCRIPTION OF ILLUSTRATIVE EMBODIMENTS

Reference now will be made in detail to the embodiments of the invention, one or more examples of which are set forth below. Each example is provided by way of explanation of the invention, not limitation of the invention. In fact, it will be apparent to those skilled in the art that various modifications and variations can be made in the present invention without departing from the scope of the appended claims. Other objects, features and aspects of the present invention are disclosed in or are obvious from the following detailed description. It is to be understood by one of ordinary skill in the art that the present discussion is a description of exemplary embodiments only, and is not intended as limiting the broader aspects of the present invention.

Unless otherwise defined herein, scientific and technical terms used in connection with the present invention shall have the meanings that are commonly understood by those of ordinary skill in the art. Further, unless otherwise required by context, singular terms shall include pluralities and plural terms shall include the singular.

The present invention provides for the manufacture of thin-layer lignocellulosic composites that include levels of isocyanate-based resins that inhibit the composite from shrinking and swelling after exposure to the elements. The invention may be applied to various types of lignocellulosic thin-layer composites to generate structural units that may be exposed to weathering by heat, moisture, air, and the like. In an embodiment, the present invention describes a method to make wood-based doorskins that are resistant to shrinking and swelling.

As used herein, "lignocellulose" comprises a material containing both cellulose and lignin. Suitable lignocellulosic materials may include wood particles, wood fibers, straw, hemp, sisal, cotton stalk, wheat, bamboo, jute, saltwater reeds, palm fronds, flax groundnut shells, hard woods, or soft woods, as well as fiberboards such as high density fiberboard (HDF), medium density fiberboard, (MDF), oriented strand board (OSB), and particle board. In an embodiment the lignocellulosic fiber is refined. As used herein, refined fiber may comprise fibers and fiber bundles that have been reduced in size from other forms of a lignocellulose substrate such as chips and shavings. In an embodiment, the lignocellulosic composites of the present invention comprise wood fiber. Refined wood fiber may be produced by softening the larger wood particles with steam and pressure and then mechanically grinding the wood in a refiner to produce the desired fiber size. In at least one embodiment, the lignocellulosic fiber is not refined.

As used herein, a thin-layer composite comprises a flat, planar structure that is significantly longer and wider than it is thick. Examples of thin-layer lignocellulosic composites include wood-based doorskins that are used to cover the frame of a door to provide the outer surface of the door. Such doorskins may be only about 1 to 13 mm thick, but may have a surface area of about 20 square feet (1.86 square meters) or more. Other thin-layer lignocellulosic products may include Medium Density Fiberboard (MDF), hardboard, particleboard, Oriented Strand Board (OSB) and other panel products made with wood. These products are normally 3 to 20 mm in thickness.

As used herein, a "lignocellulose composite" comprises a product produced by bonding lignocellulose fibers by heat and pressure. Such composites use a resin to promote bonding of the lignocellulose fibers. For example, lignocellulosic composite products may include HDF, MDF, hardboard, particleboard, OSB, and other panel products.

In an embodiment, the lignocellulosic composite is substantially free of added wax. As used herein, the term "added wax" is intended to include wax added to the mixture as a distinct component. Similarly, as used herein, "substantially free of added wax" is intended to include composites having no wax, as well as composites having a negligible amount of wax at concentrations that would not materially affect the composites, where the wax is a part of a different component of the mixture, for example the tackifier and/or release agent. For example, a composite having less than about 0.4% wax may be encompassed by the term "substantially free of added wax." In some embodiments, the composite is free of added wax. In some embodiments, various components, such as, for example, the tackifier or the release agent, may include certain amounts of wax. Embodiments in which the tackifier and/or the release agent include wax are considered to be substantially free of added wax.

In an optional embodiment, the lignocellulosic composite mixture further comprises at least one type of wax. For example, the mixture may comprise up to about 2% by weight of wax. In one embodiment, the wax is present in an amount between about 0.1 % and about 1 % by weight. In an embodiment, about 0.5% by weight wax is used.

The wax may impart additional short-term water repellency to the wood composite. The type of wax used is not particularly limited, and waxes standard in the art of wood fiber processing may be used. Generally, the wax should be stable to the temperatures used for pressing the wood/resin mixture into a thin layer, increase the water repellency of the wood, and not adversely affect the aesthetics or subsequent processing (such as priming or gluing the wood composite). Thus, the wax may be a natural wax or synthetic wax, generally having a melting point in the range of about 120° F (49° C) to about 180° F (82° C). Waxes used may include, but are not limited to, paraffin wax, polyethylene wax, polyoxyethylene wax, microcrystalline wax, shellac wax, ozokerite wax, montan wax, emulsified wax, slack wax, and combinations thereof.

The lignocellulosic mixture of the present invention may further include at least one tackifier. As used herein, the term "tackifier" is intended to include those compounds typically used in the adhesive industry to impart and/or improve the stickiness of adhesives. In the present invention, a tackifier may be blended into the mixture prior to pressing the mixture to form the present thin-layer lignocellulosic composites.

Without being bound by theory, it is believed that the tackifier enhances the interaction of the lignocellulosic fibers and the isocyanate resins, while enabling release of the composites from the dies after pressing.

Tackifiers contemplated as useful in the present invention include those tackifiers known in the adhesive industry. Suitable tackifiers include one or more tackifiers selected from rosins, lignins, hydrogenated rosins, hydrocarbons, hydrogenated hydrocarbons, pure monomers, hydrogenated pure monomers, terpene resins, and water-based dispersions of each of these. Lignosulfates, polyvinylalcohol resins, and acrylic resins are also contemplated as useful tackifiers in accordance with the present invention.

Examples of rosins and hydrogenated rosins (either fully or partially hydrogenated) include, but are not limited to, gum rosins, wood rosins, and tall oil rosins. Examples of hydrocarbons and hydrogenated hydrocarbons (either fully or partially hydrogenated) include, but are not limited to, C5 aliphatic hydrocarbon resins, such as trans-1,3-pentadiene, cis-1,3-pentadiene, 2-methyl-2-butene, dicyclopentadiene, cyclopentadiene, and cyclopentene; C9 aromatic hydrocarbons, such as vinyl toluenes, dicyclopentadiene, indene, methylstyrene, styrene, and methylindenes; and C5/C9 aliphatic/aromatic hydrocarbons, such as any combination of C5 aliphatic hydrocarbons and C9 aromatic hydrocarbons. Examples of terpene resins include, but are not limited to, thermoplastic terperene phenolic resins, terpene phenolic resins, polyterpene resins, styrenated terpene resins, and beta-pinene.

In the present invention, tackifiers may be added to the mixture at a concentration of between about 0.1% and about 5 wt %, in other embodiments between about 1% to about 2 wt %, and in some embodiments at a concentration of about 1.5 wt %.

As described herein, the lignocellulosic mixtures of the present invention are pressed into thin-layers using flat or molded dies at conditions of elevated temperature and pressure. The mixture is initially formed into a loose formed mat, and the mat is placed in the die press. Because the composite includes amounts of resin that are sufficient to increase the water resistance of the composite mixture, the composite may stick to the surface of the dies that are used to press the mat into the resultant thin layer composite. Thus, in an embodiment, the method includes steps to reduce sticking of the thin-layer composite to the dies.

In an embodiment, the method includes exposing the lignocellulosic composite mixture to a release agent prior to pressing the composite between the dies. In an embodiment, the release agent comprises an aqueous emulsion of surfactants and polymers. In one embodiment, the release agent is not a wax. For example, the release agent may comprise compounds used in the doorskin manufacturing industry such as, but not limited to, PAT®7299/D2 or PAT®1667 (Wurtz GmbH & Co., Germany).

The release agent may be added directly to the lignocellulosic composite mixture as an internal release agent prior to pre-pressing the mixture into a loose formed mat. Alternatively and/or additionally, the release agent may be sprayed on the surface of the mat before the mat is pressed into a thin layer.

Where the release agent is added directly to the mixture as an internal release agent, the amount of release agent added may range from about 0.1 to about 4 wt % of the mixture, in other embodiments between about 0.25 wt % to about 3 wt %, in other embodiments between about 0.5 wt % to about 1.5 wt %. In one embodiment, about 0.8 wt % release agent is used.

Where the release agent is sprayed onto a surface of the mat, the amount of release agent sprayed onto the mat surface may comprise from about 0.1 to about 8.0 grams solids per square foot (about 1.1 to about 86.1 grams per square meter) of mat surface. In another embodiment, the amount of release agent sprayed on the mat surface may comprise about 4 grams solids per square foot (about 43 grams per square meter) of mat surface. The release agent may be applied as an aqueous solution. In an embodiment, an aqueous solution of about 25% release agent is applied to the mat surface. When the thin-layer composite comprises a doorskin, the release agent may be applied to the surface of the mat that corresponds to the surface that will become the outer surface of the doorskin.

The selected release agent(s) should be release agents that do not interfere with subsequent processing of the resultant thin-layer composites, for example, priming and/or gluing of the final product. Release agents will typically migrate to the surface of a composite during pressing and remain at or on the surface. Some release agents, such as fatty acid release agents, are known to migrate and then interfere with subsequent processing of the composite. Release agents contemplated as useful in the present invention should include those that would not significantly interfere with subsequent processing.

In an embodiment, the thin-layered lignocellulosic composite is colored. For example, in one embodiment, the release agent may comprise a pigment. In this way, an even coloring is applied to the thin- layered lignocellulosic composite. In some embodiments, a tinted release agent would facilitate subsequent priming or painting of the door.

Thus, the thin-layer lignocellulosic composites of the present invention may comprise wood fibers as well as a tackifier and/or a release agent. For example, in an embodiment, the present invention comprises a wood composite comprising a mixture of: (i) no more than 98 wt % of a wood fiber, wherein the wood fiber has a predetermined moisture content of at least about 4%; (ii) at least about 1 wt % of an organic isocyanate resin; (iii) at least about 0.1 wt % of a tackifier; and (iv) optionally, at least about 0.1 % internal release agent by weight and/or at least about 0.1 grams release agent per square foot (about 1.1 grams per square meter) on the surface of the composite.

Other methods may be used to reduce sticking of the lignocellulosic composite to the dies used for making the resultant thin- layer composite. Thus, in another embodiment, at least one surface of the die used to press the mat is exposed to an anti-bonding agent. In an embodiment, exposing the die to an anti-bonding agent may comprise coating at least one of the dies used to press the mat with an anti-bonding agent. In an embodiment, coating the die may comprise baking the anti-bonding agent onto the die surface.

In an embodiment, the release agent is not the same as an anti-bonding agent. The release agent comprises a compound that will not interfere with subsequent processing of the resulting thin-layer composite. In contrast, the anti-bonding agent may comprise compositions known in the art of pressing wood composites as being effective in preventing sticking to the pressing dies, but that may be problematic if included as part of the composite.

For example, in an embodiment, the anti-bonding agent used to coat the die surface can be one or more of silane, silicone, siloxane, fatty acids, and polycarboxyl compounds. Thus, the anti-bonding agent used to coat the die surface may comprise anti-bonding agents known in the art of die pressing such as, but not limited to, CrystalCoat MP-3 13 and Silvue Coating (SDC Coatings, Anaheim, CA), lso-Strip-23 Release Coating (ICI Polyurethanes, West Deptford, NJ), aminoethylaminopropyltrimethoxysilane (Dow Corning Corporation), or the like.

For thin-layer doorskins, the die that is coated with the anti-bonding agent may correspond to the die used to press the outside surface of the doorskin. Alternatively, both dies may be coated with an anti-bonding agent. In an embodiment, the amount of anti-bonding agent used to coat the die surface may range in thickness from about 0.0005 to about 0.010 inches (i.e., about 0.0127 mm to about 0.254 mm). Thus, in one embodiment, the amount of anti-bonding agent used to coat the die surface comprises about 0.003 inches (i.e., about 0.0762 mm).

In some embodiments, the step of coating at least one die with an anti-bonding agent may comprise including multiple coats of bonding agent on the at least one die. For example, the at least one die may include 1, 2, 3, 4, 5, 6, 7, 8, 9 or more coats of anti-bonding agent.

Similarly, when at least one coat of anti-bonding agent is applied to the at least one die the application may not be necessary between each pressing step. For example, when pressing cycles are conducted on a regular basis, such as daily in a manufacturing facility, the anti-bonding agent may only need to be applied periodically. In some embodiments, the application may be hourly, daily, every couple of days, weekly, biweekly, monthly, some combinations thereof, etc.

In an embodiment, coating the die comprises baking the anti-bonding agent onto the die surface. For example, in one embodiment, the step of baking the anti-bonding agent onto the die surface may comprise the steps of: (i) cleaning the die surface substantially free of dirt, dust and grease; (ii) spraying from about 0.0005 to about 0.010 inches (about 0.5 to about 10 mils or about 0.0127 to about 0.254 mm) of a 50% solution of the anti-bonding agent onto the die; and (iii) baking the die at greater than 300 °F (149 °C) for about 1 to 4 hours.

In an embodiment, the step of exposing the pre-pressed mat to at least one release agent and/or anti-bonding agent may comprise adding an internal release agent and/or spraying one side of the mat with a release agent and also coating at least one die surface with an anti-bonding agent. In this embodiment, the side of the mat coated with the release agent may be the surface opposite to the surface of the mat exposed to the coated die.

In an embodiment, the step of exposing the pre-pressed mat to at least one release agent and/or anti-bonding agent may comprise adding an internal release agent and/or spraying one side of the mat with a release agent and also coating at least one die surface with an anti-bonding agent. In this embodiment, the side of the mat coated with the release agent is the surface opposite to the surface of the mat exposed to the coated die.

The thin-layered lignocelluiosic composites of the present invention may comprise a range of fiber compositions. Thus, in an embodiment, the lignocelluiosic composite mixture comprises about 80 wt% to about 98 wt% fiber.

The thin-layered wood composites of the present invention may comprise lignocelluiosic fiber comprising a range of moisture levels. In an embodiment, the method does not require dehydrating the lignocelluiosic fiber prior to treatment with the resin. Thus, in an embodiment, the lignocellulosic fiber comprises from about 4% to about 15% moisture content by weight. In another embodiment, the lignocellulosic fiber may comprise from about 8% to about 13% moisture by weight. In another embodiment, the lignocellulosic fiber may comprise about 10% moisture by weight, in other embodiments, about 9%.

In some embodiments, it may be desirable to spray additional moisture onto the mixture prior to pressing the mixture to facilitate the interaction of the isocyanate resin and the lignocellulosic fibers.

The organic isocyanate resin used may be aliphatic, cycloaliphatic, or aromatic, or a combination thereof. Monomeric, oligomeric, and polymeric isocyanates are contemplated as useful in the present invention. In an embodiment, the isocyanate may comprise diphenylmethane diisocyanate (MDI) or toluene diisocyanate (TDI) such as Lupranate®M20FB Isocyanate (BASF Corporation, Wyandotte, MI). For example, in an embodiment, the isocyanate comprises diphenylmethane-4,4'-diisocyanate. Or, in an embodiment, the isocyanate is selected from the group consisting of toluene-2,4-diisocyanate; toluene-2,6-diisocyanate; isophorone diisocyanate; diphenylmethane-4,4'-diisocyanate; 3,3'-dimethyldiphenylmethane-4,4'-diisocyanate; m - phenylene diisocyanate; p-phenylene diisocyanate; chlorophenylene diisocyanate; toluene-2,4,6-triisocyanate; 4,4',4"-triphenylmethane triisocyanate; diphenyl ether 2,4,4'-triisocyanate; hexamethylene-1,6-diisocyanate; tetramethylene-1,4-diisocyanate, cyclohexane-1,4-diisocyanate; naphthalene-1,5-diisocyanate; 1-methoxyphenyl-2,4-diisocyanate; 4,4'-biphenylene diisocyanate; 3,3'-dimethoxy-4,4'-biphenyl diisocyanate; 4,4'- dimethyldiphenylmethane-2,2',5,5'-teaisocyanate; 3,3'-dichlorophenyl-4,4'-diisocyanate; 2,2',5,5'-tetrachlorodiphenyl-4,4'-diisocyanate; trimethylhexamethylene diisocyanate; m-xylene diisocyanate; polymethylene polyphenylisocyanates; and mixtures thereof.

A range of isocyanate resin levels may be used to make the thin-layer composites of the present invention. Thus, in an embodiment, the mixture used to form the composite may comprise from about 1 % to about 5 wt % resin solids, in some embodiments about 2% to about 4 wt %. In another embodiment, the mixture may comprise about 3 wt % resin solids.

A range of isocyanate resin levels may be used to make the thin-layer composites of the present invention. Thus, in an embodiment, the mixture used to form the composite may comprise from about 3% to about 20%, in other embodiments from about 4% to about 15% by weight resin solids. In another embodiment, the mixture may comprise between 5% and 9% by weight resin solids. In one embodiment, the mixture may comprise about 8% by weight resin solids. In other embodiments, there is no significant improvement in moisture-induced shrinking or swelling when greater than about 10% by weight resin is included.

The conditions used to form the thin-layer composite include compressing the mixture at elevated temperature and pressure for sufficient time to allow the isocyanate resin to interact with the wood fibers such that the resultant thin-layer composite has a predetermined resistance to moisture. The exact conditions used will depend upon the equipment used, the exterior environment (e.g., temperature, elevation), the manufacturing schedule, the cost of input resources (e.g., starting materials, electric power), and the like. Also, varying the temperature may allow for changes to be made in the pressure used or the time of pressing; similarly, changes in pressure may require adjustment of the time and/or temperature used for pressing the thin-layer composites of the present invention.

A range of temperatures may be used to promote interaction of the isocyanate resin with the lignocellulosic fibers in the mixture. In an embodiment, the temperature used to press the mixture (or preformed mat) into a thin-layer composite may range from about 250 °F (121 °C) to about 400 °F (204 °C). In another embodiment, the temperature used to press the mixture (or preformed mat) into a thin-layer composite may range from about 280 °F (138 °C) to about 350 °F (177 °C). Or, a temperature that is in the range of from about 310 °F (154 °C) to about 330 °F (166 °C) may be used.

Similarly, the levels of the pressure applied during the pressing of the thin-layer composite may vary depending on a variety of factors, such as the nature of the thin-layer composite that is being formed, the equipment being used, environmental conditions, production capabilities, and the like. Thus, in an embodiment, the pressure during the pressing step may range from about 2500 psi (about 176 kg/cm²) to about 150 psi (about 10.5 kg/cm²). In another embodiment, the pressure may be applied in a step-wise manner. In another embodiment, the pressure during the pressing step ranges from about 1200 psi (about 84.3 kg/cm²) for about 5 to 20 seconds followed by 500 psi (about 35.16 kg/cm²) for 20 to 80 seconds. For example, in one embodiment, the pressure during the pressure step ranges from about 1200 psi (about 84.3 kg/cm²) for about 10 seconds to about 500 psi (about 35.16 kg/cm²) for about 50 seconds.

The thin-layer lignocellulosic composites of the present invention have increased resistance to moisture-induced shrinkage and swelling. As used herein, increased resistance to moisture comprises reduced shrinking and/or swelling of the thin-layer composite when the composite is exposed to conditions of low and high moisture, respectively, as compared to thin lignocellulosic composites made by other methods, or using non-isocyanate resins. The present thin-layer lignocellulosic composites have a moisture content after press of between about 4% and about 8 wt %, in some embodiments between 5% and about 7 wt %.

Thus, in an embodiment, when thin-layer composites of the present invention are exposed to an atmosphere where the moisture level is low, the composite of the present invention exhibits less shrinkage than thin-layer composites made with other resins. Also, in an embodiment, when thin-layer composites of the present invention are exposed to an atmosphere where the moisture level is high, the composite of the present invention exhibits less swelling than thin-layer composites made with other resins.

For example, in an embodiment, the thin-layer composite comprises up to 25% less linear expansion and thickness swelling after being immersed for 24 hours in 70 °F (21 °C) water than a thin-layer composite comprising comparable levels of an alternate resin, either isocyanate resins or non-isocyanate resins. Also in an embodiment, the predetermined resistance to moisture comprises a thickness swelling of less than 15% after being immersed for 24 hours in water at 70 °F (21 °C).

In another embodiment, the thin-layer composite comprises up to 50% less linear expansion and thickness swelling after being immersed for 24 hours in 70° F (21 °C) water than a thin-layer composite comprising comparable levels of an alternate (non-isocyanate) resin, such as urea formaldehyde. Also in an embodiment, the predetermined resistance to moisture comprises a thickness swelling of less than 15% after being immersed for 24 hours in water at 70° F (21° C).

Also in an embodiment, doorskins made by the methods of the present invention are significantly less dense than doorskins made using traditional formaldehyde-based resins. Thus, in an embodiment, the thin-layer lignocellulosic composites of the present invention comprise a density of between about 48 pounds per cubic foot (about 769.0 kg/m³) and about 62 pounds per cubic foot (about 993.4 kg/m³), in some embodiments less than about 60 pounds per cubic foot (about 962 kg/m³). In another embodiment, the thin-layer lignocellulosic composites of the present invention may comprise a density of less than 55 pounds per cubic foot (about 881.5 kg/m³).

The present invention provides for the manufacture of thin-layer lignocellulosic composites that include levels of isocyanate-based resins that protect the composite from shrinking and swelling upon exposure to the elements. The invention may be applied to various types of lignocellulosic thin-layer composites to generate structural units that may be exposed to weathering by heat, moisture, air, and the like. In an embodiment, the present invention describes a method to make wood- based doorskins for exterior use that are resistant to shrinking and swelling.

The present invention also comprises thin-layer lignocellulosic composites made by the methods of the invention.

Embodiments of the present aspect of the invention comprise products such as panels for composite doors and doors made using such panels. Thus, one embodiment of the present invention may comprise a product having a thin-layer lignocellulose composite that comprises a region of increased thickness to provide at least one raised surface, such that the raised surface comprises the appearance of wooden planking and/or wooden trim. The raised surface may comprise a lignocellulose composite plant-on structure in communication with the thin-layer lignocellulose composite. Alternatively and/or additionally, the raised surface may be formed by making at least one cut in the thin layer composite such that the portion of the composite next to the cut-out region comprises a raised surface. In alternate embodiments, the cut-out portion may comprise grooves or other types of hollowing of the thin-layer lignocellulose composite.

The product may comprise any building structure for which it may be desired to emulate a surface having the appearance of at least one of wooden planking or wooden trim. For example, the thin-layer lignocellulose composite may comprise a surface of a door panel. In one embodiment, the panel may comprise a panel for a garage door.

Embodiments of the present invention may also comprise doors comprising a plurality of panels, wherein at least one panel comprises a thin-layer lignocellulose composite comprising a region of increased thickness to provide at least one raised surface, such that the raised surface comprises the appearance of wooden planking and/or wooden trim. The raised surface may comprise a lignocellulose composite plant-on in communication with the thin-layer lignocellulose composite, and/or the raised surface may be formed by cutting grooves or other types of hollowing of the thin-layer lignocellulose composite. In one embodiment, the door may comprise a garage door.

As used herein, a "plant-on" comprises a structure that may be adhered to, or "planted-on" the inner or outer surface of a planar object to provide a raised surface. In one embodiment, the plant-on structure may comprise a decorative trim. The plant-on structure may be made of a material that is compatible with the surface to which it is being adhered. For example, for a lignocellulose door or panel, a plant-on may comprise a lignocellulose composite. The plant-on structure may have a variety of shapes or forms. In one embodiment, the plant-on structure may be about 3/4 inch (19 mm) thick and rectangular in shape. Or, a plant-on may comprise a lignocellulosic composite structure that is 1/2 inch (13 mm) thick and oval or round in shape.

As used herein, a cut out portion comprises a type of cut or gouge made in a surface. For example, a flat or flush door skin may have grooves that are about 1/16 inch (1.6mm) deep and 3/4 inch (19mm) wide routed in the door skin. The grooves may be substantially linear, or they may be shaped to form a decorative molding.

Also, as used in describing the various surfaces of the thin-layer composites (e.g., door skins), the term "outer surface" refers to the surface of the thin-layer composite that is exposed on either face of a composite door panel, and the term "inner surface" refers to the surface that is adjacent to the frame and inner core of the panel. In contrast, the term "outside surface" or "outside facing surface" refers to the surface of the panel that is (or is designed to be) facing the outside of a building, and the term "inside surface" or "inside facing surface" refers to the surface of the garage panel that is (or that is designed to be) facing the inside of the building. Also, a substantially flat surface comprises a surface that may have some grain, texture, or some other pattern into the surface, but that does not comprise regions of high relief. In contrast, a raised surface comprises a design that stands out, or projects from the surface.

Thus, the thin-layer lignocellulosic composites of the present invention may comprise wood fibers as well as wax and/or a release agent.

Between 1% and 15% by weight fiberglass is incorporated in the mixture, among other reasons, to further improve the linear expansion of the present thin-layer composites. In some embodiments, between about 3% and 6% by weight fiberglass may be added. In still other embodiments, about 5% by weight fiberglass may be added to the mixture.

The plant-on attached to the thin layer composite, and/or the groove or other hollowing cut into the thin-layer composite, may be used to provide the outer surface of a door panel with a pattern. The pattern may provide a single-paneled door with a desired design feature. Alternatively, the pattern may be coordinated with other panels of a multi-paneled door so as to create a door having the appearance of a single panel door. The raised surface provided by the plant-on and/or the grooves may be used to form a garage door having multiple horizontal panels that has the appearance of a single panel spanning the vertical axis of the garage door.

For example, embodiments of the present invention may comprise products having a plurality of plant-ons attached to the surface of the thin layer composite and/or grooves or other types of cut-out portions cut or formed into the surface of the thin-layer composite. The plurality of plant-ons and or grooves may comprise a repeating pattern. Alternatively and/or additionally, plant-ons or grooves positioned on the surface of one panel may be coordinated with the pattern of plant-ons or grooves on other panels used to form a pattern that extends over multiple panels.

The plant-ons may be positioned on a door comprising a substantially flat, or flush thin layer composite door skin. Alternatively, the plant-ons may be positioned on a door skin that has been cut out or routed to have grooves or some other design.

The plant-on structure may be in direct communication with the outer surface of the thin-layer composite structure. Alternatively, and/or additionally, a plant-on structure may be in direct communication with the inner surface of the thin-layer composite structure. In one embodiment, the outer or inner surface in communication with the plant-on corresponds to the outside surface of the door. Or, the outer or inner surface in communication with the plant-on may correspond to the inside surface of the door. Thus, a plant-on may be adhered to the outside facing surface of the garage door, or the inside facing surface of the garage door, or to both inside and outside facing surfaces of the garage door.

The thin-layer composite and the plant-on may both be made of the same lignocellulose material. In one embodiment, a lignocellulosic material comprises a lignocellulosic fiber and a resin. For example, the lignocellulose material used for the plant-ons and the thin-layer composite to which the plant-on is attached may comprise medium density fiberboard made with, for example, a melamine-formaldehyde resin.

In some cases, the plant-ons are only used for the outside surface of the door panel or door. The thin-layer used on the composite that does not comprise a plant-on structure may comprise a material that is the same as, or different than, the material used for the thin-layer composite that comprises the plant-on. Also, because the inside of the door is not as exposed to the elements as the outside of the door, a thin- layer composite that is less weather resistant may be used. In an embodiment, the thin-layer used on the face of the door panel that does not comprise a plant-on (e.g., the inside door skin) is also a lignocellulose composite. For example, an HDF or an MDF thin-layer composite may be used for the inside door skin.

The plant-ons may be adhered onto the thin-layer composite that will form the outer surface of the door using a polyvinyl acetate glue or a hot-melt glue. Other adhesives, such as double-sided adhesive tape may also be used. Additionally, and/or alternatively, the plant-ons may be positioned using fasteners such as, for example, nails or screws. Also, a sealant may be used to prevent delamination of the applied plant-ons from the panel. In one example embodiment, a silicone sealant, such as an acrylic silicone caulk, may be used. Also, both the thin-layer lignocellulose composite and the plant-on may comprise a resin. Thus, in one embodiment, the plant-on may be bonded to the thin-layer composite by pressing the plant-on onto the thin-layer composite such that the two composites form a singular composite and the plant-on becomes part of the thin-layer composite door skin.

By having the thin-layer composite and the plant-ons formulated from the same material, there may be reduced stress at the point of attachment of the plant-ons since both materials will exhibit the same physical characteristics. For example, when made from the same material, both the thin-layer panel and the plant-on may shrink or swell in response to changes in moisture and/or temperature in a similar fashion, resulting in reduced stress at the point of plant-on attachment as the door is exposed to environmental weathering.

The plant-ons may be a variety of shapes and sizes such that they stand out from the surface of the thin-layer lignocellulose composite door skin to provide a raised surface or relief. In various alternative embodiments, the plant-ons may range from about 1/16 to about 2 inches (1.6 - 51mm) in thickness, or from about 1/8 inch to 1 inch (3.2 - 25mm) in thickness, or from about 1/4 inch to 3/4 inch (6.4 - 19mm) in thickness. In one example embodiment, the plant-on may be about 3/8 inch (9.5mm) thick.

As described above, the thin layer composite may comprise cutout portions as a means to provide a raised surface. In one embodiment, the cut-out portions may be substantially linear, to appear as spaces between plank boards. For example, grooves may be spaced apart in a regular fashion across the surface of the thin-layer composite. Or the cutout portions may be non-linear in shape, such that the raised portions appear as decorative moldings. In one embodiment, the cut-out portions are grooves that may range from about 1/16 to 1/8 inches (1.6 - 3.2mm) deep into the surface of the thin layer composite and from about 1/16 to 1 inch (1.6 - 25mm) wide across the groove. In an embodiment, grooves about 1/16 inch (1.6mm) deep into the surface of the thin-layer lignocellulose composite and about 3/4 inch (19mm) wide across may be used. Also, the spacing between the cut-out portions may be varied. Where the raised surface is designed to appear as planking, the grooves may be spaced apart in a regular fashion. In one example embodiment, grooves may be spaced about four to eight inches (102 - 203mm) apart.

The thin-layer composite comprising a raised surface may comprise a variety of thickness ranges based in part on the method used to make the raised surface. For example, where the thin-layer composite is cut out at least in part, a thicker composite may be used. In alternate embodiments, where a portion of the thin-layer composite is cut out, the thin layer composite may range from about 1/8 inch to about 1 inch (1.6 - 25mm), or from about 1/4 inch to about 1/2 inch (6.4 - 13mm) in thickness. Alternatively, where plant-ons are used to form the raised surface, the thin layer composite may be somewhat thinner. For example, where plant-ons are used to provide a raised surface, and the thin-layer composite is not cut out, the thin-layer composite may range in thickness from about 1/8 inch to about 1 inch, (3.2 - 25mm) or from about 1/4 inch to about 1/2 inch (6.4 - 13mm).

The doors and door panels of the present invention may also comprise a core material emplaced within, and bounded by, the frame and the two thin-layer composites that form the inside and outside surfaces of the panel. The core may be made of a variety of materials. The core may, for example, comprise synthetic polymer foam. Thus, the core may comprise an expanded polystyrene (EPS) foam or a polyurethane foam. Alternatively laminated veneer lumber (LVL) or cardboard may be used to at least partly fill the core. In other embodiments, the doors and/or door panels are substantially hollow such that the core comprises a substantial proportion of air.

The core material may comprise a density similar to the density of wood. In one embodiment, expanded polystyrene having a density of from about 1.0 to about 1.5 pounds per cubic foot (pcf) (16 - 24 kg/m³) is used. In this way, the composite doors and door panels of the present invention may have the same "feel" as a wood door. For example, the composite door panel and/or door may sound like a wood door. Also, the composite door and/or door panel may have a weight that is similar to a solid wood door.

In one embodiment, the door panel may comprise translucent panels, e.g., windows made of glass, or plexiglass, or the like, inserted within the perimeters of the frame. The surface surrounding the glass panels may be flush with the outer surface of the panel, or it may comprise a plant-on or other type of trim to accentuate the window pane.

The present invention also comprises processes to make products such as composite doors and door panels having a raised surface or high relief design. In one embodiment, such doors and door panels may be used for garage doors.

A process for making a thin-layer lignocellulose composite comprising a region of increased thickness to provide at least one raised surface, such that the surface comprises the appearance of at least one of wooden planking or wooden trim has been discussed above. The method may comprise the steps of (a) preparing at least one thin-layer lignocellulose composite comprising a substantially flat surface and at least one of the following: (b) making at least one cut into the substantially flat surface of the composite to provide a raised surface, or (c) attaching at least one thin-layer lignocellulose plant-on structure to the surface of the thin-layer lignocellulose composite to form a raised surface. The cut-out portion may comprise grooves or other types of hollowing of the thin-layer lignocellulose composite.

The process may further comprise the steps of: (i) assembling a frame for a panel; and (ii) positioning the thin-layer composite on the frame to form at least part of the outer surface of the panel. In one embodiment, step (i) is performed prior to step (a) above, and step (ii) is performed prior to steps (b) and/or (c) above, such that the thin-layer composite is assembled on a frame prior to positioning the plant-on and/or making any cuts in the thin-layer surface. The panel may comprise a panel for a door. In one embodiment, the panel comprises a panel for a garage door.

In one embodiment, the raised surface is positioned on a thin-layer composite that comprises the outside surface of a panel. Additionally, a plant-on may be adhered to the surface of the door that will be the inside surface of a panel, or to both the outside and the inside surface of a panel.

The process may, in one embodiment, further comprise placing the frame on a second thin-layer substrate to form an enclosed panel prior to positioning the thin-layer composite that is to be treated to provide a raised surface. In one embodiment, the second thin-layer substrate comprises a side of the door that does not require a plant-on. Where the second thin-layer substrate does not require a plant-on, the thin-layer used on the second face of the garage door panel may comprise a material that is the same as, or different than, the material used for the face of the panel comprising the plant-on. In one embodiment, the thin-layer used on the second face of the garage door panel is a lignocellulose composite. For example, a high density fiberboard thin-layer composite may be used for the door panel that does not comprise a plant-on.

Also, in one embodiment, a core material may be emplaced within, and bounded by, the frame and the two thin-layer composites that form the inside and outside surface of the door panel. The core may be made of a variety of materials. The core may, for example, comprise a synthetic polymer foam. Thus, the core may comprise an expanded polystyrene (EPS) foam or a polyurethane foam. Alternatively, other core materials such as cardboard or LVL may be used. Or the core may be substantially hollow, such that it is filed with air.

The present invention also comprises a method of forming a product, as defined in claim 4.

In one embodiment, the raised surface provided by the plant-on and/or the cut-out portion of the thin-layer lignocellulose composite may be used to provide the outer surface of a door panel with a pattern. The pattern may provide a single-paneled door with a desired design feature. Alternatively, the pattern may be coordinated with other panels of a multi-paneled door so as to create a door having the appearance of a single panel door. For example, the raised surface provided by the plant-on and/or the cut-out portions may be used to form a garage door having multiple horizontal panels that has the appearance of a single panel spanning the vertical axis of the garage door.

The plant-ons may be positioned on a door comprising a substantially flat, or flush thin layer composite door skin such as those described above.

The thin-layer composite and the plant-on may both be made of the same lignocellulose material. For example, the lignocellulose material used for the plant-ons and the thin-layer composite to which the plant-on is attached may comprise medium density fiberboard made according to the previously discussed methods.

In some cases, the plant-ons are only used for the outside surface of the door panel or door. The thin-layer used for the surface of the door that does not comprise a plant-on structure may comprise a material that is the same as, or different than, the material used for the thin-layer composite that comprises the plant-on. In one embodiment, the thin-layer used on the face of the door panel that does not comprise a plant-on (e.g., the inside door skin) is also a lignocellulose composite. For example, an HDF or an MDF thin-layer composite may be used for the inside door skin. In some situations, because the inside of the door is not as exposed to the elements as the outside of the door, a thin-layer composite that is less weather resistant may be used.

The plant-ons may be adhered onto the thin-layer composite using a polyvinyl acetate glue or a hot-melt glue. Other adhesives, such as double-sided adhesive may also be used. Additionally, and/or alternatively, the plant-ons may be positioned using small fasteners such as, for example, nails or screws. Also, a sealant may be used to prevent delamination of the applied plant-ons from the panel. In one example embodiment, an acrylic silicone caulk sealant may be used. Also, both the thin-layer lignocellulose composite and the plant-on may comprise a resin. Thus, in one embodiment, the plant-on may be bonded to the thin-layer composite by pressing the plant-on onto the thin-layer composite such that the two composites form a singular composite and the plant-on becomes part of the thin-layer composite door skin.

The plant-ons may be a variety of shapes and sizes such that they stand out from the surface of the garage door to provide raised surface or relief. In various alternative embodiments, the plant-ons may range from about 1/16 inch to 2 inches (1.6 - 51mm) in thickness, or from about 1/8 inch to 1 inch (3.2 - 25mm) in thickness, or from about 1/4 inch to 3/4 inch (6.4 - 19mm) in thickness. In one example embodiment, the plant-on may be about 3/8 inch (9.5mm) thick.

As described above, the thin layer composite may comprise cutout portions as a means to form a raised surface. In one embodiment, the cut-out portions may be substantially linear, to appear as spaces between plank boards. For example, grooves may be spaced apart in a regular fashion across the surface of the thin-layer composite. Or the cut-out portions may be non-linear in shape, such that the raised portions appear as decorative moldings. In one embodiment, the cut-out portions are grooves that may range from about 1/16 to 1/8 inch (1.6 - 3.2mm) deep into the surface of the thin layer composite and from about 1/4 to 1 inch (6.4 - 25mm) wide across the groove. In an embodiment, grooves about 1/16 inch (1.6mm) deep and about 3/4 inch (19mm) wide across may be used. Also, the spacing between the cut-out portions may be varied. Where the raised surface is designed to appear as planking, the grooves may be spaced apart in a regular fashion. In one example embodiment, grooves may be spaced about four to eight inches (102 - 203mm) apart.

The thin-layer composite comprising a raised surface may comprise a variety of thickness ranges based in part, on the method used to make the raised surface. For example, where the thin-layer composite is cut out at least in part, a thicker composite may be used. In an embodiment, where a portion of the thin-layer composite is cut out, the thin layer composite may range from about 1/8 inch to about 1 inch (3.2 - 25mm), or from about 1/4 inch to about 1/2 inch (6.4 - 13mm) in thickness. Alternatively, where plant-ons are used to form the raised surface, the thin layer composite may be somewhat thinner. For example, where plant-ons are used to provide a raised surface, and the thin-layer composite is not cut out, the thin-layer composite may range from about 1/16 inch to about 1/2 inch (1.6 - 13mm) in thickness, or from about 1/8 inch to about 1/4 inch (3.2 - 6.4mm) in thickness.

The frame may comprise at least two vertical stiles and two horizontal rails and a thin-layer composite comprising the inner face of the door. To provide an interlocking junction between adjacent panels of the garage door, the rails may be banded with pieces of pine or other types of wood to provide a means to have adjacent panels interlock. The band may include a protruding element (i.e., a tongue), or the pine band may include a groove so that the protruding element on the end of one garage panel may be inserted into a groove on another panel to provide an almost seamless, interlocking junction between the two panels. In one embodiment, the frame is made using LVL.

Once assembled, the panel may be exposed to conditions of elevated temperature and pressure to facilitate adhering the panel parts to one another. The panel may then be primed. Also, the process may include the step of placing windows in the door. The window panes may be made of glass, or plexiglass, or the like. The part of the panel surrounding the glass panels may be flush with the outer surface of the panel, or it may comprise a plant-on or other type of trim to accentuate the window pane. Finally, the panel may be assembled to form a garage door. The door may be further decorated with hardware such as handles, knobs, knockers, straps, clavos, and the like.

Thus, the present invention comprises products, such as door panels and doors, made using a thin-layer lignocellulose composites made in accordance with the present invention that comprise a region of increased thickness to provide at least one raised surface, such that the surface comprises the appearance of wooden planking and/or wooden trim. The raised surface may comprise a lignocellulose composite plant-on structure in communication with the thin-layer lignocellulose composite. Alternatively, and/or additionally, the raised surface may be formed by making cuts in a portion of the thin-layer lignocellulose composite to thereby provide a raised surface in a portion of the composite that is adjacent to the cut-out portion.

The plant-on structures and/or the cut-out portions may be positioned to provide the door panel or door with a unique design. Because both the surface of the panel and the plant-on are made from a lignocellulose composite, the plant-on may be bonded to the door panel in such a manner as to become part of the door skin surface. Also, the doors may have the look and feel of solid wood doors.

Several methods have been described herein to produce wood composites that exhibit increased resistance to moisture uptake and loss. It is believed that swelling and/or shrinking of wood is, at least partially, the result of water reacting with hydroxyl groups present in cellulose and hemicellulose. Thus, high moisture levels increase the amount of water bound to the wood fiber. Alternatively, in low humidity, water is lost from the wood fibers.

An aspect of the present invention is concerned with methods to employ low concentrations of isocyanate resins to improve the moisture-resistance of thin-layer lignocellulosic composites, such as, but not limited to, wood doorskins. Isocyanate resins such as diphenylmethane-4,4'-diisocyanate (MDI) and toluene diisocyanate (TDI) resin are highly effective in modifying the reactive groups present on cellulose fibers to thereby prevent the fibers from reacting with water. It is believed that the isocyanate forms a chemical bond between the hydroxyl groups of the wood cellulose, thus forming a urethane linkage.

In the present invention, a thin-layer wood composite that is resistant to water is provided with resin contents of between about 1% and about 5% and in some embodiments at levels between about 2% and about 4%. Doorskins are generally on the order of 1 to 5 mm in thickness, with a total surface area of 20 square feet (i.e., 1.86 square meters). When such thin-layer wood composites made with isocyanate resin are prepared using conventional pressing methods, the high resin levels cause the wood composite to stick to the pressing die used to prepare the doorskin after only a few pressing cycles.

Figure 1 shows an overview of a general method used to prepare doorskins. Generally, a selected wood starting material is ground to prepare fibers of a uniform size and the appropriate amount of wax added. At this point the preparation may be stored until further processing. The fiber/tackifier blend is then mixed with an appropriate binder resin (e.g., using atomization), until a uniform mixture is formed. It is also common to add the resin to the fiber prior to storage of the fiber.

The mixture may then be formed into a loose formed mat which is pre-shaped using a shave-off roller and pre-compressed to a density of about 6-8 pounds per cubic foot (96 - 128 kg/m³). After further trimming to the correct size and shape, the pre-pressed mat is introduced into a platen press, and compressed between two dies under conditions of increased temperature and pressure. For example, standard pressing conditions may comprise pressing at 320 °F at 1200 psi for 10 seconds followed by 50 seconds at 500 psi (i.e., about 160 °C at 84.3 kg/cm² for 10 seconds followed by 50 seconds at 35.2 kg/cm²). Generally, a recessed (female) die is used to produce the inner surface of the doorskin, and a male die shaped as the mirror image of the female die is used to produce the outside surface of the skin. Also, the die which is forming the side of the doorskin that will be the outer surface may include an impression to create a wood grain pattern or texture. After cooling, the resulting doorskin is mounted onto a doorframe using a standard adhesive and employing mounting methods standard in the art.

In an embodiment (Figure 2), the present invention describes a method for making a thin-layer wood composite having increased water resistance comprising forming a wood composite mixture 2 comprising: (i) a refined wood fiber 4 having a predefined moisture content of about 4% to about 15%; (ii) about 0.1% to about 5.0% tackifier; (iii) between about 1.0% and about 5 wt % of an organic isocyanate resin; and (iv) optionally, at least about 1 wt % of an internal release agent (Figure 2(a)). The mixture may be prepared in bulk using standard blowline blending of the resin and fibers. Or, blenders 9 having a means for mixing 3 such as a paddle or the like, may be used.

Next, the wood composite mixture may be formed into a loose formed mat in a forming box. The mat is then pre-shaped using a shave- off roller (not shown in Figure 2) and precompressed using a roller or some other type of press 7 (Figure 2(b)). The specific density of the mat may vary depending on the nature of the wood composite being formed, but generally, the mat is formed to have a density of about 6 to 8 pounds per cubic foot (i.e., 96.2-128.1 kg per cubic meter). After further trimming of the mat to the correct size and shape, at least one surface of the mat may be exposed to additional release agent 8 by spraying the release agent onto the surface of the mat 6 using a spray nozzle 11 (Figure 2(c)). Also, shown in Figure 2 are conveyors 5 and 13 as a means for transferring the wood composite from one station to another. It is understood that other means of supporting or transferring the thin-layer wood composite from one station to another, or supporting the composite during the processing steps may be used.

The mat 6 may then be placed between a male die 14 and a female die 12, and pressed at an elevated temperature and pressure and for a sufficient time to further reduce the thickness of the thin-layer composite and to allow the isocyanate resin to interact with the wood fibers (Figure 2(d)). As described above, it is believed that by heating the wood composite in the presence of the resin, the isocyanate of the resin forms a urethane linkage with the hydroxyl groups of the wood cellulose. Replacement of the hydroxyl groups of the cellulose with the urethane linkage prevents water from hydrating or being lost from the cellulose hydroxyl groups. Thus, once the resin has cured, a doorskin having a predetermined resistance to moisture is formed. As described above, in an embodiment, one of the dies may be coated with an anti-bonding agent. Figure 2 shows an embodiment in which the female die 12 is coated on its inner surface with an antibonding agent 10.

In alternative embodiments, both dies (12 and 14) are coated with anti-bonding agent. For example, this embodiment may be preferred where both die surfaces do not have a grain pattern, but are smooth. Or, in an embodiment, both inner die surfaces may be coated with an anti-bonding agent, and the use of a release agent to coat the mat may vary depending upon the particular wood composite being prepared. Or, in an embodiment, the method may employ a release agent on the surface of the mat, without coating of the dies. In yet another embodiment, the method may employ an internal release agent in the mat, without coating of the dies.

Subsequently, the doorskin is allowed to cool (Figure 2(e)) and then further processed (sizing and priming) prior to being applied to a doorframe.

Thus, the invention describes using a release agent and/or anti-bonding agent to prevent the thin-layer wood composite from sticking to the pressing dies during production.

The release agent and/or anti-bonding agent used to prevent the mat from sticking to the dies during production may be applied to the mat in various ways. Generally, when the mat is used to produce a standard doorskin, one of the dies comprises a recess and is described as the female die. Referring to Figure 2, usually the female die 12 is positioned underneath the lower surface 18 of the mat, which is the surface of the mat that is adhered to the underlying doorframe (i.e., the inner surface). The other (upper) surface of the mat 16 corresponds to the side of the doorskin that will be on the outside of the door. Often, this side of the doorskin will include a grain texture to enhance the decorative effect. The die 14 used to press the upper side of the mat (i.e. the eventual outside of the door) may be termed the male die. Thus, the male die includes a protruding portion that is the mirror image of the recess on the female die, and optionally, a grain-like pattern on the surface of the die.

In one embodiment, an anti-bonding agent is coated onto the bottom (female) die. Depending on the actual anti-bonding agent used, the coating may be baked onto the bottom die. In this way, the coated die may be used several times before recoating with additional anti-bonding agent. For example, in an embodiment, the step of baking the anti-bonding agent onto the die surface comprises the steps of (i) cleaning the die surface substantially free of any dirt, dust or grease; (ii) spraying about 0.003 inches (3 mils; 0726 mm) of a 50% solution of the anti-bonding agent onto the die; and (iii) baking the die at over 300 °F (149 °C) for about 1-4 hours. In an embodiment, the step of cleaning the die comprises cleaning the die surface with a degreaser; wire brushing to remove solids; wiping the die surface with a solvent (such as acetone); and buffing with a cotton pad. The anti-bonding agent is then applied to provide a 3 mil thickness; and the dies heated to bake the coating onto the die. In some embodiments, the die may be coated with multiple layers of anti-bonding, with the baking step occurring after only the final coat or after only some, but not all of the coats.

Under suitable conditions, the anti-bonding agent that is baked onto the die (or dies) is stable enough with respect to the pressing conditions such that the die(s) can be used for over 2000 pressing cycles prior to requiring another coating with additional anti-bonding agent. Anti-bonding agents that are suitable for baking onto the die surface include Crystalcoat MP-3 13 and Silvue (SDC Coatings, Anaheim, CA), ISO-Strip-23 Release Coating (ICI Polyurethanes, West Deptford, NJ), aminoethlyaminopropyltrimethoxysilane (Dow Corning Corporation), or the like.

Although a preferred method to facilitate removal of the doorskin from the die uses a die coated with anti-bonding agent, other equivalent methods to facilitate nonsticking of the wood composite to the die may be incorporated into the methods of the present invention. For example, to facilitate release of the doorskin, the die(s) may be nickel plated, covered with a ceramic layer, or coated with fluorocarbons.

As described above, a release agent may be sprayed onto one of the surfaces of the pre-pressed mat prior to the mat being pressed between the dies. For example, and referring again to Figure 2, a release agent 8 may be sprayed onto the upper surface 16 of the mat 6 which is exposed to the male die 14. Preferably, the release agent 8 sprayed directly onto the surface of the mat is a release agent that is compatible with the wood and resin making up the composite. Preferably, the release agent sprayed on the wood comprises compounds such as PAT®-7299/D2, PAT®-1667 (Wurtz GmbH & Co., Germany), and the like.

The amount of release agent sprayed onto at least one side of the mat may range from 0.1 to 8.0 grams solids per square foot (1.1 to 86.1 grams per square meter) of mat. For example, the release agent may be sprayed onto the mat as a 25% aqueous solution. In an embodiment, the amount of release agent sprayed onto at least one side of the mat may comprise about 4 grams solids per square foot (i.e., 43.05 grams per square meter) of mat sprayed as a 25% aqueous solution.

The release agent used to coat the mat is distinct from the anti-bonding agent used to coat the die surface(s). The anti-bonding agent used to coat the die surface(s) generally can be one or more of silane, silicone, siloxane, fatty acids, and polycarboxyl compounds that are known to be effective coating agents. These anti-bonding agents, however, are not always suitable for spraying directly on the wood mat (or incorporating into the wood composite) since they may interfere with later finishing of the wood product by priming and/or painting.

Referring now to FIG. 3, the garage doors 19 shown may comprise multiple composite panels 21 , 23, 25, and 27, separated at junctures 22, 24, and 26. In FIG. 3 panel 23 is outlined to show the extent of the panels. Thus, it can be seen that the door may be continuous across its horizontal axis (see e.g., lower surface 29 and upper surface 31), but may be comprised of separate panels across its vertical axis (see e.g., left side 33 and right side 35). Thus, as shown in the exploded view of FIGS. 3A and 3B, although the adjacent panels 21, 23, 25, and 27 appear to form a single unified piece, there is actually a junction 22, 24, and 26, between the panels. In addition, the panels may be fashioned so that one panel may interlock with another door panel. For example, as illustrated in the exploded view shown in FIG. 3A, the seam 22 between panels 21 and 23 may comprise a protruding portion or tongue 76 on one panel, that fits into a groove 78 on an adjacent panel.

FIG. 3 shows an embodiment wherein multiple plant-ons have been positioned on the surface of the outer door skin of a garage door. By the positioning of various plant-ons on the outer surface 20 of the door panel, the overall appearance of the door is not that of four horizontal panels, but of two single-panel swing doors. For example, plant-ons 28 (FIG. 3) may span the vertical length of the door, and mesh almost seamlessly at junctions 22, 24, and 26, to appear as a single vertical trim on the face of the door. Also, diagonally placed plant-ons 32 provide a single, unified design feature to create the impression that the door shown in FIG. 3 is actually two single paneled doors that may swing open, rather than a roll-up door made of four horizontal panels (21, 23, 25, and 27). Also, hardware pieces such as handles 52 may be used to further create the impression that the door shown in FIG. 3 is actually two single paneled doors that may swing open, rather than a roll-up door made of four horizontal panels. Even horizontal plant-ons 30, although they may not span different panels, provide a design that is coordinated with the other plant-ons so as to create the impression that the door shown in FIG. 3 is actually two single-paneled swing doors.

Both the outer surface 20 of the garage door panel, and the plant-ons (e.g., 28, 30, and 32) may be made of a lignocellulose composite. For example, the thin-layer composite forming the outer surface and the plant-ons may both be made of the same lignocellulose material. In one embodiment, the lignocellulose material may comprise medium density fiberboard made using an isocyanate resin.

Referring again to FIG. 3, using a lignocellulose material allows for patterns simulating wood grain 56 to be included as part of the surface of the garage door. As used herein, a thin layer lignocellulose composite is substantially flat, and thus alone, does not comprise a raised surface. Because the plant-ons and the thin-layer composite used for the outer surface of the door are made of lignocellulose, the grain pattern 56 may be formed using dies etched with a grain pattern to form the thin-layer composite 20 and/or the plant-on (e.g., 28, 30, and 32).

Also, using a lignocellulose substrate to form the plant-ons and the thin-layer composite used as the outer surface of the door, allows for priming and painting of the garage door in a manner similar to solid wood. Thus, a variety of patterns and colors may be used with the composite garage doors of the present invention.

The plant-ons may be a variety of shapes and sizes such that they stand out from the surface of the garage door to provide raised surface or relief. In various alternative embodiments, the plant-ons may range from about 1/16 inch to 2 inches (1.6 - 51mm), or from about 1/8 inch to 1 inch (3.2 - 25mm), or from about 1/4 inch to 3/4 inch (6.4 - 19mm) in thickness 62 (FIG. 3). In one example embodiment, the plant-on may be about 3/8 inch (9.5mm) thick. The width 66 and length 64 (FIG. 3) of the plant-ons may vary depending upon the size of the door panel and the size of the trim required. In alternate embodiments, the plant-ons may range from about 1/4 inch to 18 inches (6.4 - 457mm) in width, or from about 1 inch to about 12 inches (25 - 305mm) in width, or from about 3 inch to about 10 inches (76 - 254mm) in width. The length of the plant-on may also vary, but generally will not be longer than the diagonal length of the panel. Also, different plant- ons on the same face of a door may be different sizes. For example, in one embodiment, the plant-ons 28, 30, and 32 used for the border shown in the door of FIG. 3 may be different sizes.

Still referring to FIG. 3, the door panel may comprise translucent panels 54 (e.g., windows) inserted within the perimeters of the frame. The surface of the garage door panel surrounding the window may be the door skin itself, or it may comprise a trim 34 to accentuate the window pane. In one embodiment, the trim may be a lignocellulose plant-on.

The panel itself may be sized to fit a standard garage door. In one embodiment, the panels are 78 to 144 inches (1980 - 3660mm) across for use as a single car garage door (e.g., FIGS. 3 and 4). Alternatively, panels may range from 192 to 216 inches across (4880 - 5490mm) for use as two car garage doors (e.g., FIGS. 5-8). Also, the vertical axis (i.e., height) for the panel may vary as needed. In one embodiment, four panels may be used for a garage door. Alternatively, three to six panels may be used for a garage door. Or, in some cases, the garage door may comprise a single panel. In some cases, panels of different sizes may be used for a single door. For example, in the case of a garage door including windows as part of the top panel, a larger top panel may be used with smaller lower panels. In one example embodiment, a top panel 24 inches (610mm) in height may be used with three 20 inch (508mm) lower panels. Or, four 21 inch (533mm) high panels may be used. For example, where the window is 16 inches (406mm) high, a 24 inch (610mm) high panel may be preferred. In contrast, a 13 inch (330mm) window may be fitted into a 21 inch (533mm) high panel.

FIGS. 4-8 show alternative embodiments of the garage doors and door panels of the present invention. For example, FIG. 4 shows the use of plant-ons 36 and 38 to outline an arched window-pane 54. Also, placement of vertical plant-ons 28, and horizontal plant-ons 30, as well as knobs 58 provide the appearance of two single-paneled swinging doors.

FIG. 5 provides a schematic illustration of a double (i.e., two vehicle) garage door of the present invention. Similar to FIGS. 3 and 4, FIG. 5 shows the use of multiple vertically placed plant-ons 40 to create the impression of vertical panels spanning the three bottom panels (23, 25, and 27) of the door. Also, placement of the outer vertical plant-ons 28 and horizontal plant-ons 30, provides the appearance of four single-paneled swinging doors 82, 84, 86, and 88.

FIG. 6 illustrates another embodiment, in which portions of a 1/4 inch (6.4mm) thin-layer flush (i.e., substantially flat) lignocellulose composite may be cut-out to create a pattern. For example, grooves 60 may be routed or formed in a 1/4 inch (6.4mm) thin-layer lignocellulose composite door skin to create a pattern resembling multiple boards placed in a parallel fashion. Thus, in FIG. 6, each panel (21, 23, 25, and 27) is cut out to provide grooves 60. In this way, the portions of the door skin that are not cut out 61 resemble plank boards laid adjacent to one another. The panel may also comprise a plant-on (e.g., 44 and 28), positioned on top of the thin-layer lignocellulose door skin that has been cut-out at least in part. Thus, the door of FIG. 6 provides the appearance of multiple planks that are laid side to side and that are bordered with a wooden trim to provide the arch design and frame of the door. The positioning of the plant-ons 28 and 44 relative to the cutout door skin 61 is shown as a perspective view in FIG. 6A. Also shown are decorative handles 48 and knobs 46 that convey the appearance that the door of FIG. 6 is made of four swinging door panels 82, 84, 86, and 88, rather than four horizontal panels 21, 23, 25, and 27.

FIG. 7 illustrates another embodiment in which portions of a 1/4 inch thin-layer (6.4mm) flush (i.e., substantially flat) lignocellulose composite are cut-out to create a pattern which is further accentuated by the positioning of plant-ons on top of the door skin. As shown in FIG. 7, grooves 60 may be routed from a 1/4 inch (6.4mm) thin-layer lignocellulose composite door skin to create a pattern resembling multiple boards 61 placed in a parallel fashion. The panel may also comprise plant-ons 28, 30, and 32 that are positioned on top of the door skin that has been cut-out at least in part. The positioning of the plant-ons 28, 30, and 32 relative to the cut-out door skin 61 is shown as an enlarged, perspective view in FIG. 7A. Thus, similar to the door of FIG. 6, the door of FIG. 7 provides the appearance of multiple planks that are laid side to side and that are bordered with a wooden trim to convey the appearance that the door of FIG. 7 made of four swinging or sliding door panels, rather than four horizontal panels 21, 23, 25, and 27.

An example embodiment showing the components of a composite garage door panel of the present invention is shown in FIG. 8. As illustrated in FIG. 8, the composite door panels of the present invention may comprise a frame comprising at least two vertical stiles 72 and two horizontal rails 74. Generally, three vertical stiles are preferred for a panel that spans the width of a single vehicle garage door and five to seven vertical stiles may be used for a panel that spans the width of a two vehicle garage door. As is known in the art, the stiles may be positioned such that two stiles provide the perimeter of the frame and the other stiles are spaced equidistant from the end stiles and from one another. For example, a panel for a single car garage door may comprise two exterior (perimeter) stiles and one center (interior) stile. The frame maybe made using LVL, although other types of lumber may also be used. The panel may also comprise a first thin-layer composite 70 comprising the inside face of the door and a second thin layer composite 20 comprising the outside face of the door. The rails 74 may be banded with pieces made of pine or other types of wood to provide a means to have adjacent panels interlock such that an extruding element (e.g., tongue) 76 on one panel may be inserted into a groove 78 on another panel to provide an almost seamless junction between the two panels.

As described herein, exemplary doors and door panels according to the present invention may comprise a core synthetic polymer 80, such as expanded polystyrene (EPS) or polyurethane foam, emplaced within, and bounded by the frame and the two thin-layer composites that form the inner and outer surfaces of the door (e.g., door skins). In one embodiment, expanded polystyrene having a density of from about 1.0 to about 1.5 pounds per cubic foot (pcf) (16 - 24 kg/m³) is used. Polymer products that may be used as the core are commercially available from Iowa EPS Products, Inc. (Des Moines, Iowa) or Plymouth Foam (Plymouth, Wis.).

The surface of the garage door facing the inside of the garage (e.g., 70, FIG. 8) may not require a design to the extent as may be desired on the outside facing surface (e.g., 20, FIG. 8) of the door. Thus, in many cases, the inside facing surface of the garage door panel may comprise a smooth surface. Or, a surface including a grain pattern to simulate natural wood may be used. The thin-layer composite used on the inside facing surface of the garage door panel may comprise a material that is the same as, or different than, the material used for the outside facing surface of the panel. For example, in certain applications, plastic or metal may be used as the inside facing surface of the garage door panel. Generally, however, the thin-layer composite used on the inside facing surface of the garage door panel is a lignocellulose composite. For example, an HDF door skin may be used for the inside facing surface of the door. In one example embodiment, a flat, 1/8 inch (3.2mm) thick, HDF door skin such as those commercially available from Georgia Pacific (Atlanta, GA), or Unilyn (Charlotte, NC) may be used for the inner garage door surface.

As shown in FIG. 8, the thin-layer composite 20 comprising the outside surface of the door may comprise a plurality of plant-ons 28, 30, and 32, to form a raised surface. As described above, the plant-ons may be a variety of shapes and sizes such that they stand out from the surface of the garage door to provide a raised surface or relief. Shown in FIG. 8 is a garage door panel having plant-ons 28, 30, and 32 adhered to the surface of the outer door skin 20 so as to provide the pattern for the garage door illustrated in FIG. 3. In one embodiment, the lignocellulose material may comprise medium density fiberboard made using an isocyanate resin.

Embodiments of the present invention also include processes to make products such as composite garage doors and garage door panels comprising a raised surface. A schematic representation of a process that may be used to make composite garage door panels and doors of the present invention is provided in FIGS. 9A and 9B.

As shown in FIG. 9A, one step of assembling a product comprising a raised surface to resemble wooden planking and/or trim may comprise making a flush panel 100. As used herein, a flush panel is a panel having a substantially flat surface. For example, to assemble a flush panel, a frame comprising two or three stiles and two rails for a single vehicle garage door, or five to seven stiles and two rails for a double vehicle garage door, may be assembled using either glue or fasteners as is known in the art 110. For example, the frame may be assembled by stapling the frame together using aluminum corrugated staples. Next, small aluminum nails may be inserted in the edges of the stiles, and a material to form a core is positioned inside the frame by inserting the nails in the edges of the foam 120. In one embodiment, an expanded polystyrene foam core is applied within the perimeter of the frame.

At this point, a glue may be applied to the frame so that the frame may be attached to the door skins 130. In one embodiment, the frame with the core in place may be sent through a roller that applies a glue to the frame. For example, in an embodiment, a polyvinyl acetate glue employing an aluminum chloride catalyst may be used to adhere the frame to the door skins.

The assembled frame may then be positioned on a thin-layer lignocellulose composite that will form the inside surface of the garage door 140 (FIG. 9A). These door skins may be smooth, or may have a grain pattern. In one embodiment, a high density fiberboard may be used.

Generally, multiple assemblies comprising a frame, core, and two flush thin-layer composite surfaces may be assembled 160 then pressed 170 to form panels. About 20 to 30 of the assembled structures may be stacked together and placed in a bag press, where they are pressed using air bags. For example, to press about 30 door panel assemblies, a pressure of about 138 to 345 kPa (20 to 50 psi) may be applied for about 60 minutes. After pressing, the door panels may be allowed to cure. Cure times may vary depending upon the glues and resins used to make the panel, as well as the type of door skin and frame that may have been used. Cure times may range from 20 minutes to as long as 48 hours. In one embodiment, a cure time of about 4 hours is used.

Once the panels have cured sufficiently, they may be trimmed to size and shaped to include a tongue or groove on the rails 180. For example, a door trim saw may be used to trim one or both rails, and one or both outer stiles. Once the panel has been appropriately trimmed to size, the rails may be fashioned to include a portion comprising either a protruding piece (e.g., a "tongue") or a groove. The tongue and groove pieces will allow the panels to interlock in a substantially seamless manner. For example, referring back to FIGS. 3 and 8, the protruding tongue 76 from the upper rail of panel 23, may insert into the groove 78 on the lower rail of panel 21, to provide an interlocking junction at 22.

At this point, and referring now to FIG. 9B, the panels may be bent to have portions of the door skin raised. Thus, the process may include the option 199 of having the flush panels bent to have portions of at least one of the door skins cut out 200. Alternatively, and/or additionally, the process includes glue alternative 299 of having the panels bent to have plant-ons applied 300.

Where the panels are to have grooves or other types of cut-out portions emplaced in the outer surface 200, the thin layer lignocellulose composite used as the outer surface may be thicker than a standard 1/8 inch (3.2mm) door skin. For example, a 1/4 inch (6.4mm) lignocellulose composite may be used. To have grooves cut into the outer door skin, a router may be used to cut grooves in the door panel at predetermined positions 200. For example, in one embodiment, grooves 1/8 inch (3.2mm) deep, and 3/8 inch (9.5mm) wide are cut in the door panel every six inches (152mm).

Once the door panels have been cured and trimmed to size 100, and if needed, part of the surface cut-out to form a pattern 200, individual plant-on structures may be placed on the upper surface of the door skin to form the design required 300 (FIG. 9B). As shown in FIG. 9B, a step may comprise making the plant-on structures that may be applied to the thin-layer lignocellulose composite door skin. To form the plant-on structures, a lignocellulose sheet of the correct thickness is prepared 310 and then cut, or torn, to the correct size 320. For example, the plant-ons may be formed from 3/8 inch (9.5mm) MDF thin-layer composite that has been cut to the correct size. In one embodiment, the plant-ons are cut manually. In an alternative embodiment, the plant-ons may be cut using a laser. More specifically, the plant-ons may be shaped using a multiple head ripsaw. For example, individual 3/8 inch (9.5mm) MDF sheets may be fed into the rip saw having a blade configuration set to generate the proper widths needed for the plant-on material.

Once the appropriate plant-ons have been prepared, the plant-on may be positioned on the thin-layer lignocellulose composite 330. In one embodiment, an adhesive may be used. For example, an isocyanate adhesive may be applied to the plant-on structure using a roller or glue spreader. Alternatively, a double-sided adhesive tape may be used. Or a combination of tape with an adhesive spray may be employed. Also, hot-melt glue, such as National Starch reactive hotmelt may be used to apply the plant-on to a thin-layer lignocellulose composite resin. For example, in one embodiment, the plant-on material is applied using a polyvinyl acetate (PVA) glue catalyzed with aluminum chloride catalyst. The PVA may be applied at a rate of 8 to 10 mils thickness (0.008-0.010 inch, 0.20-0.25mm). Also, the plant-on may be further secured using a fastener, such as a nail, aluminum brad rivet, tack, or other fasteners known in the art.

Once the plant-on has been positioned on the panel, the panel may be subjected to pressure such that the plant-on is fixed onto the outer surface of the door panel 340. For example, the panel may be pressed for at least one hour at 20 psi (138 kPa) air pressure using a bag press. Because the plant-on is made of the same lignocellulose material as the door skin to which it is attached, the surface plant-on will be compatible with the surface of the door skin such that the outer door skin will comprise a single structure having raised portions provided by the plant-on.

At this point the panels may be primed with primer 400. The process may further include the option 499 of sending the panels to have windows emplaced in the panel 500. To insert windows, an opening may be cut in the panel surface using, for example, a routing window cutout machine 510. The window frames may then be installed in the opening, caulked, and fastened together with screws 520. Decorative trim may then be put in place 520. The decorative trim may be pre-made trim such as plastic trim. Or, the decorative trim may comprise a plant-on.

Once the raised surfaces have been added to the panel, and if needed, windows emplaced, the process may include the option 599 of sending the panels to be assembled into doors 600. The pressed panel may be painted as required 610. Using a lignocellulose substrate to form the plant-ons and the thin-layer composite used as the outer surface of the door allows for priming and painting of the garage door in a manner similar to solid wood. Thus, a variety of patterns and colors may be used with the composite garage doors of the present invention. Although a variety of paint types may be used, a waterborne all-acrylic exterior latex finish with a UV inhibitor may be employed to provide a wide range of color choice, relative ease of application and substantial durability. Once the panels have been painted, they may be assembled as doors 620. Or, panels may be assembled as doors and then painted as needed.

The present invention is also concerned with methods to employ isocyanate resins to improve the moisture-resistance of thin-layer lignocellulosic composites, such as, but not limited to, wood doorskins. Isocyanate resins such as diphenylmethane-4,4'-diisocyanate (MDI) and toluene diisocyanate (TDI) resin are highly effective in modifying the reactive groups present on cellulose fibers to thereby prevent the fibers from reacting with water. It is believed that the isocyanate forms a chemical bond between the hydroxyl groups of the wood cellulose, thus forming a urethane linkage.

Efforts to develop isocyanate resins for thin-layer wood composites are described in U.S. Pat. No. 3,440,189, describing the use of isocyanate resin and a basic catalyst, U.S. Pat. No. 4,100,138, describing the use of an isocyanate and a polyether polyol binder, as well as U.S. Pat. No. 4,359,507, describing use of isocyanates mixed with ethylene carbonate and propylene carbonate as a binder. Also, U.S. Pat. No. 6,620,459 describes a method for impregnating wood substrates with an isocyanate resin by dipping the wood in the resin followed by subsequent polymerization steps, and U.S. Pat. Nos. 4,388,138 and 4,396,673 describe use of a binder of polyisocyanate and a wax release agent. U.S. Pat. No. 5,344,484 describes the use of low-temperature pressing to prepare isocyanate-bonded wood composites described as having high surface strength but porous enough such that adhesives can bond the treated thin-layer composite to an underlying wood frame. U.S. Pat. No. 5,344,484 describes that such wood composites include 1 to 4% isocyanate resin. Still, it has been found that such low levels of resin do not provide consistent levels of moisture resistance to thin-layer wood composites.

To provide a thin-layer wood composite that is resistant to water, resin contents of greater than 5%, in some embodiments at levels of about 6%, up to about 15%, are required. However, there are problems when manufacturing thin-layer lignocellulosic composites using isocyanate- based resins at concentrations greater than 5%. For example, doorskins are generally on the order of 2 to 5 mm in thickness, with a total surface area of 20 square feet (i.e., 1.86 square meters). When such thin-layer wood composites made with 10% isocyanate resin are prepared using conventional pressing methods, the high resin levels typically cause the wood composite to stick to the pressing die used to prepare the doorskin after only a few pressing cycles.

As described herein, the present invention describes the use of isocyanate resins to prepare wood composites. One of the advantages of using isocyanate resins rather than formaldehyde crosslinked resins is that less energy is needed to dry the wood fiber prior to pressing the mat. As described herein, traditional phenol-formaldehyde resins are not compatible with wood having a water content much greater than 8%, as the water tends to interfere with the curing process. Also, excess moisture in the wood fiber can cause blistering when pressed with melamine-formaldehyde resins or urea-formaldehyde resins. Thus, for wood having a moisture content of greater than 8%, the wood must be dried for the curing step, and then re-hydrated later. In contrast, isocyanate-based resins are compatible with wood having a higher water content and thus, curing with isocyanate-based resins may obviate the need for the drying and the re-hydrating steps associated with formaldehyde-based resins. Moreover, the use of isocyanate resins in place of formaldehyde-based resins results in a reduction of formaldehyde resins. The present concentration of isocyanate resins results in lower volatile organic compound (VOC) emissions. Accordingly, the present composites provide synergistic environmental improvements over previous thin-layer lignocellulosic composites.

In an embodiment, the press time and temperature may vary depending upon the resin used. For example, using a toluene diisocyanate (TDI) resin as opposed to diphenylmethane diisocyanate (MDI) resin may shorten the press time by as much as 10%. Generally, when using isocyanate resins, very high temperatures are not required; thus, isocyanate resins are associated with decreased energy costs and less wear on the boiler or other energy generator. Still, composites made at very low temperatures do not display sufficient resistance to moisture to be commercially useful. Thus, the temperature used for pressing may range from 250 °F to 400 °F (121 °C to 204 °C), or more preferably, between 280 °F and 350 °F (138 °C to 177 °C). In an embodiment, ranges between 310 °F (154 °C) to about 330 °F (166 °C) are preferred.

The pressure used during pressing may be constant, or varied in a step-wise fashion. Depending upon the selected temperature and pressure conditions used for pressing, the total pressing may range from 30 seconds to 2 minutes or more. Thus, the pressure during the pressing step may include ranges from about 2500 psi (about 176 kg/cm²) to about 150 psi (about 10.5 kg/cm²). Or, the pressure may be applied in a stepwise manner. For example, the pressure during the pressing step may range from about 1200 psi (about 84.3 kg/cm²) for about 5 to 20 seconds followed by 500 psi (about 35.16 kg/cm²) for 10 to 80 seconds. In one embodiment, the pressure during the pressure step ranges from about 1200 psi (about 84.3 kg/cm²) for about 10 seconds to about 500 psi (about 35.16 kg/cm²) for about 30 seconds.

Preferably, wood composites made by the method of the invention comprise significantly less linear expansion and swelling than wood composites made by conventional methods. Thus, doorskins made by the method of the present invention exhibit about 50% less linear expansion and thickness swelling than composite doorskins made with formaldehyde-based resins of the same content (such as, for example, 3% melamine-urea-formaldehyde doorskins) when boiled in water for 2 hours. Also, doorskins made by the present invention exhibit about 50% less linear expansion than non-isocyanate based doorskins when immersed in water for 24 hours at 70 °F (21.1 °C), a standard test used in the industry (ASTM D1037).

As described above, the thin-layer lignocellulosic composites of the present invention comprise a predetermined thickness, such that the resultant composite comprises a flat planar structure. In an embodiment, the predetermined thickness ranges from about 0.085 inches to about 0.250 inches (about 2.16 mm to about 6.35 mm). In an alternate embodiment, the predetermined thickness of the thin-layer composite may range from about 0.110 to about 0.130 inches (about 2.79 to about 3.30 mm).

In some embodiments, the thin-layer lignocellulosic composites of the present invention comprise a predetermined thickness, such that the resultant composite comprises a flat planar structure. In an embodiment, the predetermined thickness ranges from 0.100 inches to 0.5 inches (2.54 mm to 13 mm). In an alternate embodiment, the predetermined thickness of the thin-layer composite may range from 0.090 to 0.385 inches (2.28 to 9.78 mm).

Also in an embodiment, doorskins made by the methods of the present invention are significantly less dense than doorskins made using traditional formaldehyde-based resins. For a doorskin that is 0.12 inches (3.05 mm) thick and has 10% melamine-urea formaldehyde resin and 1.5% wax, the density is about 58 pounds per cubic foot (930 kg/m³). In contrast, doorskins of the present invention (3% MDI resin; 0.8% internal press release) may have a density as low as about 48 pounds per cubic foot (769.0 kg/m³).

### EXAMPLE

Various parameters that would be expected to improve the stability of doorskins exposed to moisture were tested, including altering the moisture content and other attributes of the wood fiber, altering the amount and type of the resin, and altering the press conditions (temperature, pressure and/or time).

Ultimately, it was found that isocyanate-based resin binders provided a wood composite that is resistant to water when resin levels of about 1 % and up to about 5% were employed. When these levels of resin were used, however, the resulting composite tended to stick to the pressing dies during manufacture.

Various methods were tried to prevent the doorskins from sticking to the dies. It was determined that the addition of a release agent to the surface of the pre-pressed mat used to make the doorskin allowed the doorskin to be removed from the male die. In additional experiments, the release agent was added directly to the composite mixture. For effective release, approximately 0.1 to 4 wt % of the release agent was required. It was found that for consistent results, about 0.25 to 3% internal release agent was preferred.

As the release agent is theoretically only required at the surface, methods to treat the surface of the doorskin were evaluated. It was found that spraying the surface of the mat with a 25% solution of PAT®-7299/D2 (Wurtz GmbH & Co., Germany) provided sufficient release agent to successfully remove the doorskin from the male die. It was further found that concentrations of release agent ranging from 0.1 to 8 grams solid per square foot (1.1 to 86.1 grams per square meter) of mat were effective (generally administered as a 25% solution). About 2-4 grams release agent solids per square foot (2.2 to 43.05 grams per square meter) of mat were found to provide consistent results, with higher concentrations providing only minimally better results.

Methods were evaluated to apply a release agent to the underside of the mat and the top surface of the bottom die for each press load. It was found, however, that treating the surface of the bottom die with an anti-bonding agent may be preferable for eliminating bonding of the mat to the bottom die. An anti-bonding agent, such as Silvue (SDC Coatings) was used to coat the surface of the female die. Initial experiments used excess anti-bonding agent to flood the surface of the die. Further testing indicated that baking the anti-bonding agent onto the surface of the female (bottom) die allowed for the die to be used multiple times prior to being retreated. To bake the anti-bonding agent onto the die, the female die was treated by (i) cleaning the surface of the die substantially free of dust, dirt and grease using a degreaser, wire brush treatment and solvent; (ii) spraying about 0.003 inches (3 mils; 0.0762 mm) of a 50% solution of the release agent onto the die; and (iii) baking the die at a temperature of about 300 °F (149 °C) to 350 °F (177 °C) for about 1-4 hours.

Thus, it was found that addition of 0.19-0.37 g.m⁻² (2-4 g per square foot) of a release agent to the upper surface of the pre-pressed mat, and baking the anti-bonding agent Silvue (SDC Coatings) onto the female (bottom) die allowed for easy removal of the doorskins having about 1 % to about 5% MDI resin from both dies easily. Additionally, it was determined that over 2000 press loads could be made prior to recoating the female die with additional antibonding agent.

The wood composites made by the method of the invention demonstrated significantly less linear expansion and swelling than wood composites made by conventional methods. Thus, doorskins made by the method of the present invention exhibited 50% less linear expansion and thickness swelling than composite doorskins made with formaldehyde based resins of the same content (e.g., 1 % melamine-urea-formaldehyde doorskins) when boiled in water for 2 hours. Also, doorskins made by the present invention exhibited 50% less linear expansion than comparable formaldehyde-based doorskins than non-isocyanate based doorskins when immersed in water for 24 hours at 70 °F (21.1 °C), a standard test used in the industry (ASTM D1037).

Also, doorskins made by the methods of the present invention were found to be significantly less dense than doorskins made using traditional formaldehyde-based resins.

Accordingly, the present methods form composites that have increased resistance to moisture-induced shrinking and/or swelling as compared to composites with similar concentrations of non-isocyanate resins. The present methods also may be used to form composites having comparable resistance to moisture-induced shrinking and/or swelling as composites having greater concentrations of isocyanate resins. The inventors, therefore, have developed methods and products demonstrating reduced emissions, while maintaining and improving the physical characteristics of the composites using concentrations previously understood to be unworkable.

The present methods also result in reduced energy costs, high-throughput production, and reduced over-all costs while maintaining the necessary moisture resistance of the composites.

It will be understood that each of the elements described above, or two or more together, may also find utility in applications differing from the types described. Although the invention has been illustrated and described as a method for high-throughput preparation of thin-layer lignocellulosic composites, such as doorskins, it is not intended to be limited to the details shown, since various modifications and substitutions can be made without departing in any way from the present invention. As such, further modifications may occur to persons skilled in the art, within the scope of the invention as defined in the claims.

## Claims

1. A method of producing a thin-layer lignocellulosic composite (20,70) having increased resistance to moisture-induced shrinking or swelling comprising:
(a) forming a lignocellulosic composite mixture (2) comprising at least one type of lignocellulosic fiber (4) comprising a moisture content of at least 4 wt %, and at least 1 wt % of an organic isocyanate resin;
(b) pre-pressing the mixture into a loose formed mat (6); and
(c) pressing the mat (6) between two dies (12, 14) at an elevated temperature and pressure and for a sufficient time further reducing the thickness of the mat (6) to form a thin-layer composite (20, 70) having a thickness of 1 mm to 24.5 mm (1 inch) and allowing the isocyanate resin to interact with the lignocellulosic fiber (4) such that the resultant thin-layer composite (20, 70) has a predetermined resistance to moisture,
**characterised in that** said lignocellulosic composite mixture (2) further comprises between 1 wt % and 15 wt % fiberglass.

2. The method according to Claim 1, wherein the lignocellulosic mixture (2) comprises 80% to 98 wt % fiber.

3. The method according to Claim 1 or 2, wherein the predetermined resistance to moisture comprises a thickness swelling of less than 15% after the resultant thin-layer composite (20, 70) has been immersed for 24 hours in water at 70 °F (21 °C).

4. A method of forming a product, comprising producing a thin-layer lignocellulosic composite (20) by the method of any preceding claim and providing at least one raised surface that comprises the appearance of wooden planking and/or trim, the raised surface being formed by a lignocellulose plant-on structure (28, 30, 32) in communication with the thin-layer lignocellulosic composite (20), and/or by making at least one hollow (60) in the thin layer composite (20) such that the portion of the composite next to the hollow comprises the raised surface.

5. A thin-layer lignocellulosic composite (20, 70) having a thickness of 1 mm to 24.5 mm (1 inch) and being formed by pressing a mat (6) between two dies (12, 14) at elevated temperature and pressure, wherein the mat (6) is formed of a mixture comprising:
at least one type of lignocellulosic fiber (4), wherein the fiber (4) comprises a moisture content of at least 4 wt% and
at least 1 wt % of an organic isocyanate resin,
**characterised in that** said mixture further comprises between 1 wt % and 15 wt % fiberglass.

6. The thin-layer lignocellulosic composite (20, 70) according to Claim 5, wherein the isocyanate comprises diphenylmethane diisocyanate or toluene diisocyanate.

7. The thin-layer lignocellulosic composite (20, 70) according to Claim 5, wherein the isocyanate comprises diphenylmethane-4,4'-diisocyanate.

8. The thin-layer lignocellulosic composite (20, 70) according to any of Claims 5 - 7, which exhibits a thickness swelling of less than 15% after being immersed for 24 hours in water at 70 °F (21 °C).

9. The thin-layer lignocellulosic composite (20, 70) according to any of Claims 5 - 8, having a thickness ranging from 0.085 inches to 0.250 inches (2.16 mm to 6.35 mm), preferably from 0.110 inches to 0.130 inches (2.79 mm to 3.30 mm); or having a thickness ranging from 0.100 inches to 0.5 inches (2.54 mm to 13mm).

10. The thin-layer lignocellulosic composite (20, 70) according to any of Claims 5-9, further comprising a density of less than 65 pounds per cubic foot (1042 kg/m³), preferably between 48 pounds per cubic foot and 62 pounds per cubic foot (769.0 kg/m³ and 993.4 kg/m³); or having a density of less than 55 pounds per cubic foot (881.2 kg/m³).

11. The thin-layer lignocellulosic composite (20, 70) according to any of Claims 5 - 10, wherein said mixture (2) comprises between 3% and 6% by weight fiberglass.

12. The thin-layer lignocellulosic composite (20, 70) according to any of claims 5 -11, wherein said mixture (2) comprises about 5% by weight fibreglass.

13. The thin-layer lignocellulosic composite (20, 70) according to any of Claims 5 - 12, wherein the lignocellulosic fiber (4) comprises wood.

14. A product comprising a thin-layer lignocellulosic composite (20) according to Claim 13 in form of a door skin and having at least one raised surface that comprises the appearance of wooden planking and/or trim, the raised surface being formed by a lignocellulose plant-on structure (28, 30, 32) in communication with the thin-layer lignocellulosic composite (20), and/or by at least one hollow (60) in the thin layer composite (20) such that the portion of the composite next to the hollow comprises the raised surface.

## Patentansprüche

1. Herstellungsverfahren für einen dünnschichtigen Lignozelluloseverbundstoff (20, 70) mit erhöhter Resistenz gegen durch Feuchtigkeit verursachtes Schrumpfen oder Quellen, wobei das Verfahren Folgendes umfasst:
(a) Bilden einer Lignozelluloseverbundstoff-Mischung (2) umfassend wenigstens eine Art von einen Feuchtigkeitsgehalt von wenigstens 4 Gew.-% aufweisenden Lignozellulosefasern (4) und wenigstens 1 Gew.-% eines organischen Isozyanatharzes;
(b) Vorpressen der Mischung in eine lose geformte Matte (6); und
(c) Pressen der Matte (6) zwischen zwei Platten (12, 14) bei erhöhter Temperatur und erhöhtem Druck und für eine ausreichende Zeit, um die Dicke der Matte (6) weiter zu verringern, um einen dünnschichtigen Lignozelluloseverbundstoff (20, 70) mit einer Dicke von 1 mm bis 24,5 mm (1 Zoll) zu bilden, und Ermöglichen einer Wechselwirkung des Isozyanatharzes mit der Lignozellulosefaser (4), so dass der resultierende dünnschichtige Lignozelluloseverbundstoff (20, 70) eine vorbestimmte Resistenz gegen Feuchtigkeit aufweist,
**dadurch gekennzeichnet, dass** die Lignozelluloseverbundstoff-Mischung (2) weiterhin zwischen 1 Gew.-% und 15 Gew.-% Glasfaser enthält.

2. Verfahren nach Anspruch 1, wobei die Lignozellulosemischung (2) 80 bis 98 Gew.-% Fasern umfasst.

3. Verfahren nach Anspruch 1 oder 2, wobei die vorbestimmte Resistenz gegen Feuchtigkeit eine Dickenquellung von weniger als 15 % umfasst, nachdem der resultierende dünnschichtige Lignozelluloseverbundstoff (20, 70) 24 Stunden lang in Wasser eingetaucht wurde bei einer Temperatur von 70 °F (21 °C).

4. Verfahren zur Herstellung eines Produkts, das Verfahren umfassend das Herstellen eines dünnschichtigen Lignozelluloseverbundstoffs (20) durch das Verfahren nach einem der vorhergehenden Ansprüche und das Bereitstellen wenigstens einer erhabenen Oberfläche, die das Aussehen einer Holzbeplankung und/oder -verkleidung umfasst, wobei die erhabene Oberfläche durch eine Lignozelluloseanpflanzstruktur (28, 30, 32) gebildet wird, die mit dem dünnschichtigen Lignozelluloseverbundstoff (20) in Verbindung steht, und/oder indem mindestens eine Vertiefung (60) in dem dünnschichtigen Lignozelluloseverbundstoff (20) derart ausgeformt wird, dass der Abschnitt des Verbundstoffs neben der Vertiefung die erhabene Oberfläche aufweist.

5. Dünnschichtiger Lignozelluloseverbundstoff (20, 70) mit einer Dicke von 1 mm bis 24,5 mm (1 Zoll), der durch Pressen einer Matte (6) zwischen zwei Platten (12, 14) bei erhöhter Temperatur und erhöhtem Druck gebildet wird, wobei die Matte (6) aus einer Mischung gebildet ist, die Folgendes umfasst:
wenigstens eine Art von Lignozellulosefasern (4), wobei die Fasern (4) einen Feuchtigkeitsgehalt von wenigstens 4 Gew.-% aufweisen und
wenigstens 1 Gew.-% eines organischen Isozyanatharzes,
**dadurch gekennzeichnet, dass** die Mischung weiterhin zwischen 1 Gew.-% und 15 Gew.-% Glasfaser enthält.

6. Dünnschichtiger Lignozelluloseverbundstoff (20, 70) nach Anspruch 5,
wobei das Isozyanat Diphenylmethandiisozyanat oder Toluoldiisozyanat umfasst.

7. Dünnschichtiger Lignozelluloseverbundstoff (20, 70) nach Anspruch 5,
wobei das Isozyanat Diphenylmethan-4,4'-diisozyanat umfasst.

8. Dünnschichtiger Lignozelluloseverbundstoff (20, 70) nach einem der Ansprüche 5 bis 7, der nach 24-stündigem Eintauchen in Wasser bei 70 °F (21 °C) eine Dickenquellung von weniger als 15 % aufweist.

9. Dünnschichtiger Lignozelluloseverbundstoff (20, 70) nach einem der Ansprüche 5 bis 8, der eine Dicke im Bereich von 0,085 Zoll bis 0,250 Zoll (2,16 mm bis 6,35 mm) aufweist, vorzugsweise von 0,110 Zoll bis 0,130 Zoll (2,79 mm bis 3,30 mm); oder eine Dicke von 0,100 Zoll bis 0,5 Zoll (2,54 mm bis 13 mm) aufweist.

10. Dünnschichtiger Lignozelluloseverbundstoff (20, 70) nach einem der Ansprüche 5 bis 9, weiterhin umfassend eine Dichte von weniger als 65 Pfund pro Kubikfuß (1042 kg/m³), vorzugsweise zwischen 48 Pfund pro Kubikfuß und 62 Pfund pro Kubikfuß (769,0 kg/m³ und 993,4 kg/m³); oder mit einer Dichte von weniger als 55 Pfund pro Kubikfuß (881,2 kg/m³).

11. Dünnschichtiger Lignozelluloseverbundstoff (20, 70) nach einem der Ansprüche 5 bis 10, wobei die Mischung (2) zwischen 3 Gew.-% und 6 Gew.-% Glasfaser umfasst.

12. Dünnschichtiger Lignozelluloseverbundstoff (20, 70) nach einem der Ansprüche 5 bis 11, wobei die Mischung (2) etwa 5 Gew.-% Glasfaser umfasst.

13. Dünnschichtiger Lignozelluloseverbundstoff (20, 70) nach einem der Ansprüche 5 bis 12, wobei die Lignozellulosefaser (4) Holz umfasst.

14. Produkt umfassend einen dünnschichtigen Lignozelluloseverbundstoff (20) nach Anspruch 13 in Form einer Türhaut und mit wenigstens einer erhabenen Oberfläche, die das Aussehen einer Holzbeplankung und/oder -verkleidung umfasst, wobei die erhabene Oberfläche durch eine Lignozelluloseanpflanzstruktur (28, 30, 32) gebildet wird, die mit dem dünnschichtigen Lignozelluloseverbundstoff (20) in Verbindung steht, und/oder durch wenigstens eine Vertiefung (60) in dem dünnschichtigen Lignozelluloseverbundstoff (20), so dass der Abschnitt des Verbundstoffs neben der Vertiefung die erhabene Oberfläche aufweist.

## Revendications

1. Procédé de production d'un composite lignocellulosique en couche mince (20,70) ayant une résistance accrue au rétrécissement ou au gonflement induit par l'humidité comprenant les étapes consistant à :
(a) former un mélange de composite lignocellulosique (2) comprenant au moins un type de fibre lignocellulosique (4) comprenant une teneur en humidité d'au moins 4 % en poids, et au moins 1 % en poids d'une résine isocyanate organique ;
(b) pré-presser le mélange en un mat formé lâche (6) ; et
(c) presser le mat (6) entre deux trémies (12, 14) à une température et une pression élevées et durant un temps suffisant réduisant en outre l'épaisseur du mat (6) pour former un composite en couche mince (20, 70) ayant une épaisseur de 1 mm à 24,5 mm (1 pouce) et permettant à la résine isocyanate d'interagir avec la fibre lignocellulosique (4) de telle manière que le composite en couche mince résultant (20, 70) a une résistance à l'humidité prédéterminée,
**caractérisé en ce que** ledit mélange de composite lignocellulosique (2) comprend en outre entre 1 % en poids et 15 % en poids de fibre de verre.

2. Procédé selon la revendication 1, dans lequel le mélange lignocellulosique (2) comprend 80 % à 98 % en poids de fibres.

3. Procédé selon la revendication 1 ou 2, dans lequel la résistance prédéterminée à l'humidité comprend un gonflement d'épaisseur de moins de 15 % après que le composite en couche mince résultant (20, 70) a été immergé durant 24 heures dans l'eau à 70°F (21°C).

4. Procédé de formation d'un produit, comprenant la production d'un composite lignocellulosique en couche mince (20) par le procédé selon l'une quelconque des revendications précédentes et de fourniture d'au moins une surface élevée qui comprend l'apparence d'un platelage en bois et/ou d'une garniture, la surface élevée étant formée par une structure de matériel de lignocellulose (28, 30, 32) en communication avec le composite lignocellulosique en couche mince (20),
et/ou en effectuant au moins un creux (60) dans le composite en couche mince (20) de telle manière que la partie du composite près du creux comprend la surface élevée.

5. Composite lignocellulosique en couche mince (20,70) ayant une épaisseur de 1 mm à 24,5 mm (1 pouce) qui est formé en pressant un mat (6) entre deux trémies (12, 14) à une température et une pression élevées, où le mat (6) est formé d'un mélange comprenant :
au moins un type de fibre lignocellulosique (4), où la fibre (4) comprend une teneur en humidité d'au moins 4 % en poids et
au moins 1 % en poids d'une résine isocyanate organique,
**caractérisé en ce que** ledit mélange comprend en outre entre 1 % en poids et 15 % en poids de fibre de verre.

6. Composite lignocellulosique en couche mince (20, 70) selon la revendication 5, dans lequel l'isocyanate comprend du diphénylméthane-diisocyanate ou du toluène-diisocyanate.

7. Composite lignocellulosique en couche mince (20, 70) selon la revendication 5, dans lequel l'isocyanate comprend du diphénylméthane-4,4'-diisocyanate.

8. Composite lignocellulosique en couche mince (20, 70) selon l'une quelconque des revendications 5 à 7, qui présente un gonflement d'épaisseur de moins de 15 % après avoir été immergé durant 24 heures dans l'eau à 70°F (21°C).

9. Composite lignocellulosique en couche mince (20, 70) selon l'une quelconque des revendications 5 à 8, ayant une épaisseur se situant dans la plage allant de 0,085 pouce à 0,250 pouce (2,16 mm à 6,35 mm), de préférence de 0,110 pouce à 0,130 pouce (2,79 mm à 3,30 mm) ; ou ayant une épaisseur située dans la plage allant de 0,100 pouce à 0,5 pouce (2,54 mm à 13 mm).

10. Composite lignocellulosique en couche mince (20, 70) selon l'une quelconque des revendications 5 à 9, comprenant en outre une densité de moins de 65 livres par pied cubique (1042 kg/m³), de préférence entre 48 livres par pied cubique et 62 livres par pied cubique (769,0 kg/m³ et 993,4 kg/m³) ; ou ayant une densité de moins de 55 livres par pied cubique (881,2 kg/m³).

11. Composite lignocellulosique en couche mince (20, 70) selon l'une quelconque des revendications 5 à 10, dans lequel ledit mélange (2) comprend entre 3 % et 6 % en poids de fibre de verre.

12. Composite lignocellulosique en couche mince (20, 70) selon l'une quelconque des revendications 5 à 11, dans lequel ledit mélange (2) comprend environ 5 % en poids de fibre de verre.

13. Composite lignocellulosique en couche mince (20, 70) selon l'une quelconque des revendications 5 à 12, dans lequel la fibre lignocellulosique (4) comprend du bois.

14. Produit comprenant un composite lignocellulosique en couche mince (20) selon la revendication 13 en forme de revêtement de porte et ayant au moins une surface élevée qui comprend l'apparence d'un platelage de bois et/ou de garniture, la surface élevée étant formée par une structure de matériel de lignocellulose (28 ,30, 32) en communication avec le composite lignocellulosique en couche mince et/ou par au moins un creux (60) dans le composite en couche mince (20) de telle manière que la partie du composite près du creux comprend la surface élevée.
